

[54] ELECTROPHOTOGRAPHIC  
PHOTOSENSITIVE MEMBER WITH  
PYRAZOLINE CHARGE TRANSPORT  
MATERIAL

[75] Inventors: **Yoshio Takasu, Tama; Shozo Ishikawa, Sayama, both of Japan**

[73] Assignees: **Canon Kabushiki Kaisha; Copyer Kabushiki Kaisha**, both of Tokyo, Japan

[21] Appl. No.: 383,629

[22] Filed: Jun. 1, 1982

[30] **Foreign Application Priority Data**

|                    |       |       |           |
|--------------------|-------|-------|-----------|
| Jun. 10, 1981 [JP] | Japan | ..... | 56-89256  |
| Jun. 15, 1981 [JP] | Japan | ..... | 56-91876  |
| Jun. 23, 1981 [JP] | Japan | ..... | 56-97764  |
| Jun. 23, 1981 [JP] | Japan | ..... | 56-97765  |
| Jun. 23, 1981 [JP] | Japan | ..... | 56-97766  |
| Jun. 23, 1981 [JP] | Japan | ..... | 56-97767  |
| Jun. 23, 1981 [JP] | Japan | ..... | 56-97768  |
| Jul. 22, 1981 [JP] | Japan | ..... | 56-114837 |
| Jul. 22, 1981 [JP] | Japan | ..... | 56-114838 |

[51] Int. Cl.<sup>3</sup> ..... G03G 5/06; G03G 5/14  
 [52] U.S. Cl. ..... 430/59; 430/58;  
       430/76; 430/77; 430/78; 548/374; 548/379  
 [58] Field of Search ..... 430/58, 59, 76, 77,  
       430/78

## [56] References Cited

## U.S. PATENT DOCUMENTS

|           |        |                                |
|-----------|--------|--------------------------------|
| 3,180,729 | 4/1965 | Klupfel et al. .               |
| 3,837,851 | 9/1974 | Shattuck et al. .              |
| 3,859,303 | 1/1975 | Katsuyama et al. .... 430/76 X |
| 4,278,746 | 7/1981 | Goto et al. .                  |
| 4,315,982 | 2/1982 | Ishikawa et al. .              |

## FOREIGN PATENT DOCUMENTS

55-2285 1/1980 Japan ..... 430/58  
 55-88065 7/1980 Japan ..... 430/59  
 1030024 5/1966 United Kingdom .

*Primary Examiner*—Roland E. Martin, Jr.  
*Attorney, Agent, or Firm*—Fitzpatrick, Cella, Harper & Scinto

[57] ABSTRACT

An electrophotographic photosensitive member is characterized by comprising a layer which contains at least one pyrazoline compound represented by the following formula (I) or (II):



wherein m and n represent 0 or 1; when both m and n are 0, X<sub>1</sub> represents a substituted or unsubstituted heterocyclic residue; R<sub>1</sub> represents a substituted or unsubstituted aryl or heterocyclic residue; R<sub>2</sub> and R<sub>3</sub> each represent hydrogen or a substituted or unsubstituted aryl or heterocyclic residue; or they form spiropyrazoline cojointly with the carbon atom to which they are linked; and R<sub>5</sub> represents hydrogen, a halogen, or a substituted or unsubstituted alkyl or aryl;

when m is 1 and n is 0,  $X_1$  represents a substituted or unsubstituted heterocyclic residue;  $R_1$  and  $R_2$  each represent a substituted or unsubstituted aryl or heterocyclic residue;  $R_3$  represents hydrogen; and  $R_4$  and  $R_5$  each represent hydrogen, a halogen, or a substituted or unsubstituted alkyl or aryl;

substituted or unsubstituted aryl or aryl, when  $m$  is 0 and  $n$  is 1,  $X_1$ ,  $R_1$ ,  $R_2$ , and  $R_3$  each represent a substituted or unsubstituted aryl or heterocyclic residue,  $R_2$  and  $R_3$  may also form spiropyrazoline cojointly with the carbon atom to which they are linked, and one of  $R_2$  and  $R_3$  can also be hydrogen but  $X_1$  is not a substituted or unsubstituted aryl unless  $R_2$  and  $R_3$  form spiropyrazoline as mentioned above; and  $R_4$  and  $R_5$  each represent hydrogen, a halogen, or a substituted or unsubstituted alkyl or aryl; if  $R_3$ ,  $R_4$ , and  $R_5$  each are hydrogen, neither  $R_1$  nor  $R_2$  is a di-substituted aminophenyl; when both  $m$  and  $n$  are 1,  $X_1$  represents a substituted

when both  $m$  and  $n$  are 1,  $X_1$  represents a substituted or unsubstituted heterocyclic residue;  $R_1$  and  $R_2$  each represent a substituted or unsubstituted aryl or heterocyclic residue; and  $R_4$  and  $R_5$  each represent hydrogen, a halogen, or a substituted or unsubstituted alkyl or aryl.



wherein  $X_2$  and  $X_3$  each represent a substituted or unsubstituted heterocyclic residue;  $R_6$  represents a substituted or unsubstituted divalent hydrocarbon residue;  $R_7$  and  $R_8$  each represent a substituted or unsubstituted aryl or heterocyclic residue; and  $R_9$  and  $R_{10}$  each represent hydrogen, a halogen, or a substituted or unsubstituted alkyl or aryl.

**9 Claims, No Drawings**



substituted or unsubstituted aryl unless R<sub>2</sub> and R<sub>3</sub> form spiropyrazoline as mentioned above; R<sub>4</sub> and R<sub>5</sub> each represent hydrogen, a halogen, or a substituted or unsubstituted alkyl or aryl; and if R<sub>3</sub>, R<sub>4</sub>, and R<sub>5</sub> are hydrogen, neither R<sub>1</sub> nor R<sub>2</sub> is a 5 di-substituted aminophenyl; when both m and n are 1, X<sub>1</sub> represents a substituted or unsubstituted heterocyclic residue; R<sub>1</sub> and R<sub>2</sub> each represent a substituted or unsubstituted aryl or heterocyclic residue; and R<sub>4</sub> and R<sub>5</sub> each represent hydrogen, a halogen, or a substituted or unsubstituted alkyl or aryl.



Formula (II) 15

20

wherein X<sub>2</sub> and X<sub>3</sub> each represent a substituted or unsubstituted heterocyclic residue; R<sub>6</sub> represents a substituted or unsubstituted divalent hydrocarbon residue; 25 R<sub>7</sub> and R<sub>8</sub> each represent a substituted or unsubstituted aryl or heterocyclic residue; and R<sub>9</sub> and R<sub>10</sub> each represent hydrogen, a halogen, or a substituted or unsubstituted alkyl or aryl. 30

#### DETAILED DESCRIPTION OF THE PREFERRED EMBODIMENT

The organic photoconductive materials or charge-transporting for use in this invention are represented by 35 the following formula (I) or (II):



Formula (I)

40

wherein m and n represent 0 or 1; when both m and n are 0, X<sub>1</sub> represents a substituted or unsubstituted heterocyclic residue; R<sub>1</sub> represents a substituted or unsubstituted aryl or heterocyclic residue; 50 R<sub>2</sub> and R<sub>3</sub> each represent hydrogen or a substituted or unsubstituted aryl or heterocyclic residue; or they form spiropyrazoline cojointly with the carbon atom to which they are linked; and R<sub>3</sub> represents hydrogen, a halogen, or a substituted or unsubstituted alkyl or aryl; when m is 1 and n is 0, X<sub>1</sub> represents a substituted or unsubstituted heterocyclic residue; R<sub>1</sub> and R<sub>2</sub> each represent a substituted or unsubstituted aryl or heterocyclic residue; 55 R<sub>3</sub> represents hydrogen; and R<sub>4</sub> and R<sub>5</sub> each represent hydrogen, a halogen, or a substituted or unsubstituted alkyl or aryl; when m is 0 and n is 1, X<sub>1</sub>, R<sub>1</sub>, R<sub>2</sub> and R<sub>3</sub> each represent a substituted or unsubstituted aryl or heterocyclic residue, R<sub>2</sub> and

R<sub>3</sub> may also form spiropyrazoline cojointly with the carbon atom to which they are linked, and one of R<sub>2</sub> and R<sub>3</sub> can also be hydrogen, but X<sub>1</sub> is not a substituted or unsubstituted aryl unless R<sub>2</sub> and R<sub>3</sub> form spiropyrazoline as mentioned above;

R<sub>4</sub> and R<sub>5</sub> each represent hydrogen, a halogen, or a substituted or unsubstituted alkyl or aryl; and if R<sub>3</sub>, R<sub>4</sub>, and R<sub>5</sub> are hydrogen, neither R<sub>1</sub> nor R<sub>2</sub> is a di-substituted aminophenyl; when both m and n are 1, X<sub>1</sub> represents a substituted or unsubstituted heterocyclic residue; R<sub>1</sub> and R<sub>2</sub> each represent a substituted or unsubstituted aryl or heterocyclic residue; and R<sub>4</sub> and R<sub>5</sub> each represent hydrogen, a halogen, or a substituted or unsubstituted alkyl or aryl.



Formula (II)

20

wherein X<sub>2</sub> and X<sub>3</sub> each represent a substituted or unsubstituted heterocyclic residue;

R<sub>6</sub> represents a substituted or unsubstituted divalent hydrocarbon residue;

R<sub>7</sub> and R<sub>8</sub> each represent a substituted or unsubstituted aryl or heterocyclic residue; and

R<sub>9</sub> and R<sub>10</sub> each represent hydrogen, a halogen, or a substituted or unsubstituted alkyl or aryl.

The heterocyclic residue represented by X<sub>1</sub>, X<sub>2</sub>, X<sub>3</sub>, R<sub>1</sub>, R<sub>2</sub>, R<sub>3</sub>, R<sub>7</sub>, or R<sub>8</sub> is selected from 2-pyridyl, 3-pyridyl, 4-pyridyl, 2-quinolyl, 4-quinolyl, 3-carbazolyl, 2-furyl, 4-imidazolyl, 4-oxazolyl, 4-thiazolyl, isoxazolyl, and the like. These heterocyclic residues may also have substituents selected from halogens (e.g., chlorine and bromine), alkyls (e.g., methyl, ethyl, n-propyl, isopropyl, n-butyl, t-butyl, etc.), alkoxy (e.g., methoxy, ethoxy, butoxy, etc.), substituted alkyls (e.g., benzyl, 2-phenylethyl,  $\alpha$ -naphthylmethyl,  $\beta$ -naphthylmethyl, 2-methoxyethyl, 3-methoxypropyl, 2-hydroxyethyl, 3-hydroxypropyl, 3-carboxypropyl, 2-chloroethyl, 2-bromoethyl, etc.), and aryls (e.g. phenyl, tolyl, xylol,  $\alpha$ -naphthyl,  $\beta$ -naphthyl, etc.).

The aryl or substituted aryl as X<sub>1</sub> is selected from phenyl, tolyl, xylol, biphenyl, chlorophenyl, dichlorophenyl, trichlorophenyl, bromophenyl, dibromophenyl, tribromophenyl, cyanophenyl, ethylphenyl, methoxyphenyl,  $\alpha$ -naphthyl,  $\beta$ -naphthyl, etc.

The aryl as R<sub>1</sub>, R<sub>2</sub>, R<sub>3</sub>, R<sub>7</sub>, or R<sub>8</sub> is selected from phenyl,  $\alpha$ -naphthyl,  $\beta$ -naphthyl, anthryl, etc. These aryls are preferred to have substituents selected from dialkylaminos (e.g., N,N-dimethylamino, N,N-diethylamino, N,N-dipropylamino, N,N-dibutylamino, 60 N,N-dipentylamino, N-methyl-N-ethylamino, N-methyl-N-propylamino, and N-ethyl-N-propylamino), cyclic aminos (e.g., morpholino, piperidino, and pyrrolidino), and alkoxy (e.g., methoxy, ethoxy, propoxy, and butoxy). Further, alkyls of the above dialkylamino and of

65 the above alkoxy each may also be substituted by a suitable atom (e.g., chlorine, bromine, or fluorine) or an organic residue (e.g., tolyl, xylol, chlorophenyl, phenyl, naphthyl, hydroxy, carboxy, cyano, or amino). Typical

examples of the aryl include dialkylaminophenyl, cyclic aminophenyl, and alkoxyphenyl, for example, 4-N,N-dimethylaminophenyl, 4-N,N-diethylaminophenyl, 4-N,N-dipropylaminophenyl, 4-N,N-dibutylaminophenyl, 4-N,N-dibenzylaminophenyl, 4-morpholinophenyl, 4-piperidinophenyl, 4-pyrrolidinophenyl, 4-methoxyphenyl, 4-ethoxyphenyl, 4-butoxyphenyl, etc.

The aryl or substituted aryl as R<sub>4</sub>, R<sub>5</sub>, R<sub>9</sub>, or R<sub>10</sub> is selected from phenyl, tolyl, xylyl, biphenyl, ethylphenyl, diethylphenyl, nitrophenyl, cyanophenyl, hydroxyphenyl, carboxyphenyl, chlorophenyl, dichlorophenyl, trichlorophenyl, bromophenyl, dibromophenyl, aminophenyl, N,N-dimethylaminophenyl, N,N-diethylaminophenyl, N,N-dibenzylaminophenyl,  $\alpha$ -naphthyl,  $\beta$ -naphthyl, etc.

The halogen atom represented by R<sub>4</sub>, R<sub>5</sub>, R<sub>9</sub>, or R<sub>10</sub> is selected from chlorine, bromine, iodine atoms, and the like, and alkyl or substituted alkyl represented by the same is selected from C<sub>1</sub>-C<sub>5</sub> alkyls such as, for example, methyl, ethyl, n-propyl, isopropyl, n-butyl, t-butyl, n-amyl, and t-amyl or from substituted alkyls such as, for example, benzyl, chlorobenzyl, dichlorobenzyl, trichlorobenzyl, bromobenzyl, methylbenzyl, dimethylbenzyl, cyanobenzyl, 2-phenylethyl,  $\alpha$ -naphthylmethyl,  $\beta$ -naphthylmethyl, vinylmethyl, 2-chloroethyl, 3-chloropropyl, 2-hydroxyethyl, 3-hydroxypropyl, 2-methoxyethyl, 3-methoxypropyl, 4-methoxybutyl, and 2-phenoxyethyl.

As examples of the substituted or unsubstituted divalent hydrocarbon residue represented by R<sub>6</sub> in formula (II) above, there may be cited arlenes such as



and aliphatic hydrocarbon residues such as (7) —CH=CH—, (8) —CH=CH—CH=CH—, (9) —CH<sub>2</sub>—, and (10) —CH<sub>2</sub>—CH<sub>2</sub>—. These divalent residues each may be substituted by a suitable atom (e.g., chlorine, bromine, or fluorine, etc.) or an organic residue (e.g., cyano, hydroxy, carboxy, nitro, amino, methyl, ethyl, propyl, butyl, benzyl, 2-phenylethyl, 2-methoxyethyl, 3-methoxypropyl, 2-hydroxyethyl, phenyl, tolyl, etc.).

In preferred embodiments of this invention, the pyrazoline compound of formula (I) above is represented by the following formula of (1) to (8):

5



(1)



(2)



(3)



(4)



(5)



(6)



(7)



(8)

In these formulae, the same symbols as in formula (I) have the same meanings as given above; R<sub>11</sub> represents a substituted or unsubstituted alkyl (e.g., methyl, ethyl, propyl, 2-hydroxyethyl, and 2-chloroethyl); R<sub>12</sub> represents hydrogen, a halogen (e.g., chlorine, bromine, or iodine), or an organic monovalent residue, including, for example, alkyls (such as methyl, ethyl, and propyl), alkoxys (such as methoxy, ethoxy, and propoxy), alkoxycarbonyls (such as methoxycarbonyl, ethoxycarbonyl, and propoxycarbonyl), and nitro; l is an integer of 1 to 4; and Z represents



or  $-\text{CH}=\text{CH}-$ , wherein  $\text{R}_{13}$  and  $\text{R}_{14}$  each represent a substituted or unsubstituted alkyl such as methyl, ethyl, propyl, 2-hydroxyethyl, or 2-chloroethyl.

Examples of suitable pyrazoline compounds represented by formula (I) are listed below.

| Compound No. | Compound name                                                                                      |
|--------------|----------------------------------------------------------------------------------------------------|
| (1)          | 1-[pyridyl-(3)]-3,5-di-(4-N,N-dimethylaminophenyl)-pyrazoline                                      |
| (2)          | 1-[pyridyl-(3)]-3,5-di-(4-N,N-diethylaminophenyl)-pyrazoline                                       |
| (3)          | 1-[pyridyl-(3)]-3,5-di-(4-N,N-dibenzylaminophenyl)-pyrazoline                                      |
| (4)          | 1-[pyridyl-(3)]-3,5-di-(4-N-ethyl-N-propylamino-phenyl)pyrazoline                                  |
| (5)          | 1-[pyridyl-(3)]-3-(4-N,N-diethylaminophenyl)-5-(4-N,N-dibenzylaminophenyl)pyrazoline               |
| (6)          | 1-[pyridyl-(3)]-3,5-di-(4-morpholinophenyl)-pyrazoline                                             |
| (7)          | 1-[pyridyl-(3)]-3,5-di-(4-piperidinophenyl)-pyrazoline                                             |
| (8)          | 1-[pyridyl-(3)]-3,5-di-(4-pyrrolidinophenyl)-pyrazoline                                            |
| (9)          | 1-[pyridyl-(3)]-3,5-di-(4-methoxyphenyl)pyrazoline                                                 |
| (10)         | 1-[pyridyl-(3)]-3,5-di-(4-ethoxyphenyl)pyrazoline                                                  |
| (11)         | 1-[pyridyl-(3)]-3-(4-N,N-diethylaminophenyl)-5-(4-methoxyphenyl)pyrazoline                         |
| (12)         | 1-[pyridyl-(3)]-3,5-diphenylpyrazoline                                                             |
| (13)         | 1-[pyridyl-(3)]-3,5-diphenyl-3-(4-N,N-diethylaminophenyl)pyrazoline                                |
| (14)         | 1-[6-methoxy-pyridyl-(2)]-3,5-di-(4-N,N-dimethylaminophenyl)pyrazoline                             |
| (15)         | 1-[6-methoxy-pyridyl-(2)]-3,5-di-(4-N,N-diethylaminophenyl)pyrazoline                              |
| (16)         | 1-[6-methoxy-pyridyl-(2)]-3,5-di-(4-N,N-dibenzylaminophenyl)pyrazoline                             |
| (17)         | 1-[6-methoxy-pyridyl-(2)]-3,5-di-(4-N,N-dipropylaminophenyl)pyrazoline                             |
| (18)         | 1-[6-methoxy-pyridyl-(2)]-3,5-di-(4-N,N-dibutylaminophenyl)pyrazoline                              |
| (19)         | 1-[6-methoxy-pyridyl-(2)]-3-(4-N,N-diethylaminophenyl)-5-phenylpyrazoline                          |
| (20)         | 1-[6-methoxy-pyridyl-(2)]-3-(4-N-ethyl-N-benzylaminophenyl)-5-(4-N,N-diethylaminophenyl)pyrazoline |
| (21)         | 1-[6-methoxy-pyridyl-(2)]-3,5-di-(4-methoxyphenyl)-pyrazoline                                      |
| (22)         | 1-[6-methoxy-pyridyl-(2)]-3-(4-N,N-diethylaminophenyl)-5-(4-methoxyphenyl)pyrazoline               |
| (23)         | 1-[6-methoxy-pyridyl-(2)]-3,5-di-(4-morpholinophenyl)pyrazoline                                    |
| (24)         | 1-[6-methoxy-pyridyl-(2)]-3,5-di-(4-piperidinophenyl)pyrazoline                                    |
| (25)         | 1-[6-methoxy-pyridyl-(2)]-3,5-di-(4-pyrrolidinophenyl)pyrazoline                                   |
| (26)         | 1-[pyridyl-(2)]-3,5-di-(4-N,N-dimethylaminophenyl)-pyrazoline                                      |
| (27)         | 1-[pyridyl-(2)]-3,5-di-(4-N,N-diethylaminophenyl)-pyrazoline                                       |
| (28)         | 1-[pyridyl-(2)]-3,5-di-(4-N,N-dibenzylaminophenyl)-pyrazoline                                      |
| (29)         | 1-[pyridyl-(2)]-3,5-di-(4-N,N-dipropylamino-phenyl)pyrazoline                                      |
| (30)         | 1-[pyridyl-(2)]-3,5-di-(4-N,N-dibutylamino-phenyl)pyrazoline                                       |
| (31)         | 1-[pyridyl-(2)]-3,5-di-(4-morpholinophenyl)-pyrazoline                                             |
| (32)         | 1-[pyridyl-(2)]-3,5-di-(4-methoxyphenyl)pyrazoline                                                 |
| (33)         | 1-[pyridyl-(2)]-3-(4-N,N-diethylaminophenyl)-5-(4-methoxyphenyl)pyrazoline                         |
| (34)         | 1-[quinolyl-(2)]-3,5-di-(4-N,N-dimethylamino-phenyl)pyrazoline                                     |

-continued

| Compound No. | Compound name                                                                                                                                                                                                                                                                              |
|--------------|--------------------------------------------------------------------------------------------------------------------------------------------------------------------------------------------------------------------------------------------------------------------------------------------|
| 5 (35)       | 1-[quinolyl-(2)]-3,5-di-(4-N,N-diethylamino-phenyl)pyrazoline                                                                                                                                                                                                                              |
| (36)         | 1-[quinolyl-(2)]-3,5-di-(4-N,N-dibenzylamino-phenyl)pyrazoline                                                                                                                                                                                                                             |
| (37)         | 1-[quinolyl-(2)]-3,5-di-(4-N-ethyl-N-propylamino-phenyl)pyrazoline                                                                                                                                                                                                                         |
| 10 (38)      | 1-[quinolyl-(2)]-3-(4-N,N-diethylaminophenyl)-5-(4-N,N-dibenzylaminophenyl)pyrazoline                                                                                                                                                                                                      |
| (39)         | 1-[quinolyl-(2)]-3,5-di-(4-morpholinophenyl)-pyrazoline                                                                                                                                                                                                                                    |
| (40)         | 1-[quinolyl-(2)]-3,5-di-(4-piperidinophenyl)-pyrazoline                                                                                                                                                                                                                                    |
| 15 (41)      | 1-[quinolyl-(2)]-3,5-di-(4-pyrrolidinophenyl)-pyrazoline                                                                                                                                                                                                                                   |
| (42)         | 1-[quinolyl-(2)]-3,5-di-(4-methoxyphenyl)-pyrazoline                                                                                                                                                                                                                                       |
| (43)         | 1-[quinolyl-(2)]-3,5-di-(4-ethoxyphenyl)pyrazoline                                                                                                                                                                                                                                         |
| (44)         | 1-[quinolyl-(2)]-3-(4-N,N-diethylaminophenyl)-5-(4-methoxyphenyl)pyrazoline                                                                                                                                                                                                                |
| 20 (45)      | 1-[quinolyl-(2)]-3,5-diphenylpyrazoline                                                                                                                                                                                                                                                    |
| (46)         | 1-[quinolyl-(2)]-5,5-diphenyl-3-(4-N,N-diethylaminophenyl)pyrazoline                                                                                                                                                                                                                       |
| (47)         | 1-[lepidyl-(2)]-3,5-di-(4-N,N-diethylaminophenyl)-pyrazoline                                                                                                                                                                                                                               |
| 25 (48)      | 1-[lepidyl-(2)]-3,5-di-(4-N,N-diethylaminophenyl)-pyrazoline                                                                                                                                                                                                                               |
| (49)         | 1-[lepidyl-(2)]-3,5-di-(4-N,N-dibenzylamino-phenyl)pyrazoline                                                                                                                                                                                                                              |
| (50)         | 1-[lepidyl-(2)]-3,5-di-(4-N-ethyl-N-propylamino-phenyl)pyrazoline                                                                                                                                                                                                                          |
| 30 (51)      | 1-[lepidyl-(2)]-3-(4-N,N-diethylaminophenyl)-5-(4-N,N-dibenzylaminophenyl)pyrazoline                                                                                                                                                                                                       |
| (52)         | 1-[lepidyl-(2)]-3,5-di-(4-morpholinophenyl)-pyrazoline                                                                                                                                                                                                                                     |
| (53)         | 1-[lepidyl-(2)]-3,5-di-(4-piperidinophenyl)-pyrazoline                                                                                                                                                                                                                                     |
| (54)         | 1-[lepidyl-(2)]-3,5-di-(4-pyrrolidinophenyl)-pyrazoline                                                                                                                                                                                                                                    |
| 35 (55)      | 1-[lepidyl-(2)]-3,5-di-(4-methoxyphenyl)-pyrazoline                                                                                                                                                                                                                                        |
| (56)         | 1-[lepidyl-(2)]-3,5-di-(4-ethoxyphenyl)pyrazoline                                                                                                                                                                                                                                          |
| (57)         | 1-[lepidyl-(2)]-3-(4-N,N-diethylaminophenyl)-5-(4-methoxyphenyl)pyrazoline                                                                                                                                                                                                                 |
| 40 (58)      | 1-[lepidyl-(2)]-3,5-diphenylpyrazoline                                                                                                                                                                                                                                                     |
| (59)         | 1-[carbazolyl-(3)]-3,5-di-(4-N,N-dimethylamino-phenyl)pyrazoline                                                                                                                                                                                                                           |
| (60)         | 1-[carbazolyl-(3)]-3,5-di-(4-N,N-diethylamino-phenyl)pyrazoline                                                                                                                                                                                                                            |
| 45           | These compounds are readily prepared by known synthetic methods, for instance, by refluxing an unsaturated ketone and a hydrazino compound represented by the following formulae (a) and (b), respectively, in alcohol in the presence of a small amount of acetic acid for several hours. |
| 55 (a)       | $\begin{array}{c} \text{R}_2 \\ \diagdown \\ \text{C}=\text{CH}-\text{C}=\text{O} \\ \diagup \\ \text{R}_3 \end{array}$                                                                                                                                                                    |
| 55 (b)       | $\text{X}_1-\text{NH}-\text{NH}_2$                                                                                                                                                                                                                                                         |
| 60           | ( $\text{R}_1$ , $\text{R}_2$ , $\text{R}_3$ and $\text{X}_1$ are as defined above)                                                                                                                                                                                                        |
| 61 (61)      | 1-[pyridyl-(3)]-3-(4-N,N-diethylaminostyryl)-4-methyl-5-(4-N,N-dimethylaminophenyl)pyrazoline                                                                                                                                                                                              |
| 62 (62)      | 1-[pyridyl-(3)]-3-(4-N,N-diethylaminostyryl)-4-methyl-5-(4-N,N-diethylaminophenyl)pyrazoline                                                                                                                                                                                               |
| 63 (63)      | 1-[pyridyl-(3)]-3-(4-N,N-diethylaminostyryl)-4-methyl-5-(4-N,N-dibenzylaminophenyl)pyrazoline                                                                                                                                                                                              |
| 64 (64)      | 1-[pyridyl-(3)]-3-(4-N-ethyl-N-propylaminostyryl)-4-methyl-5-(4-N-ethyl-N-propylaminophenyl)pyrazoline                                                                                                                                                                                     |

-continued

- (65) 1-[pyridyl-(3)]-3-(4-N,N-diethylaminostyryl)-4-methyl-5-(4-N,N-dibenzylaminophenyl)pyrazoline  
 (66) 1-[pyridyl-(3)]-3-(4-morpholinostyryl)-4-methyl-5-(4-morpholinophenyl)pyrazoline  
 (67) 1-[pyridyl-(3)]-3-(4-piperidinostyryl)-4-methyl-5-(4-piperidinophenyl)pyrazoline  
 (68) 1-[pyridyl-(3)]-3-(4-pyrrolidinostyryl)-4-methyl-5-(4-pyrrolidinophenyl)pyrazoline  
 (69) 1-[pyridyl-(3)]-3-(4-methoxystyryl)-4-methyl-5-(4-methoxyphenyl)pyrazoline  
 (70) 1-[pyridyl-(3)]-3-(4-ethoxystyryl)-4-methyl-5-(4-ethoxyphenyl)pyrazoline  
 (71) 1-[pyridyl-(3)]-3-(4-N,N-diethylaminostyryl)-4-methyl-5-(4-methoxyphenyl)pyrazoline  
 (72) 1-[pyridyl-(3)]-4-methyl-5,5-diphenyl-3-(4-N,N-diethylaminostyryl)pyrazoline  
 (73) 1-[pyridyl-(3)]-4-methyl-3,5-di-(4-N,N-diethylaminophenyl)pyrazoline  
 (74) 1-[pyridyl-(3)]-4-methyl-3,5-di-(4-N,N-dibenzylaminophenyl)pyrazoline  
 (75) 1-[pyridyl-(3)]-4-methyl-3,5-di-(4-morpholinophenyl)pyrazoline  
 (76) 1-[pyridyl-(3)]-3-(4-N,N-diethylaminostyryl)-4-ethyl-5-(4-N,N-diethylaminophenyl)pyrazoline  
 (77) 1-[pyridyl-(3)]-3-(4-N,N-diethylaminostyryl)-4-ethyl-5-(4-N,N-diethylaminophenyl)pyrazoline  
 (78) 1-[pyridyl-(3)]-3-(4-N,N-dibenzylaminostyryl)-4-ethyl-5-(4-N,N-dibenzylaminophenyl)pyrazoline  
 (79) 1-[pyridyl-(3)]-3-(4-N-ethyl-N-propylaminostyryl)-4-ethyl-5-(4-N-ethyl-N-propylaminophenyl)pyrazoline  
 (80) 1-[pyridyl-(3)]-3-(4-N,N-diethylaminostyryl)-4-ethyl-5-(4-N,N-dibenzylaminophenyl)pyrazoline  
 (81) 1-[pyridyl-(3)]-3-(4-morpholinostyryl)-4-ethyl-5-(4-morpholinophenyl)pyrazoline  
 (82) 1-[pyridyl-(3)]-3-(4-piperidinostyryl)-4-ethyl-5-(4-piperidinophenyl)pyrazoline  
 (83) 1-[pyridyl-(3)]-3-(4-pyrrolidinostyryl)-4-ethyl-5-(4-pyrrolidinophenyl)pyrazoline  
 (84) 1-[pyridyl-(3)]-3-(4-methoxystyryl)-4-ethyl-5-(4-methoxyphenyl)pyrazoline  
 (85) 1-[pyridyl-(3)]-3-(4-ethoxystyryl)-4-ethyl-5-(4-ethoxyphenyl)pyrazoline  
 (86) 1-[pyridyl-(3)]-3-(4-N,N-diethylaminostyryl)-4-ethyl-5-(4-methoxyphenyl)pyrazoline  
 (87) 1-[pyridyl-(3)]-4-ethyl-5,5-diphenyl-3-(4-N,N-diethylaminostyryl)pyrazoline  
 (88) 1-[pyridyl-(3)]-4-ethyl-3,5-di-(4-N,N-diethylaminophenyl)pyrazoline  
 (89) 1-[pyridyl-(3)]-4-ethyl-3,5-di-(4-N,N-dibenzylaminophenyl)pyrazoline  
 (90) 1-[pyridyl-(3)]-4-ethyl-3,5-di-(4-morpholinophenyl)pyrazoline  
 (91) 1-[pyridyl-(3)]-3-(4-N,N-dimethylaminostyryl)-4-benzyl-5-(4-N,N-diethylaminophenyl)pyrazoline  
 (92) 1-[pyridyl-(3)]-3-(4-N,N-diethylaminostyryl)-4-benzyl-5-(4-N,N-diethylaminophenyl)pyrazoline  
 (93) 1-[pyridyl-(3)]-3-(4-N,N-dibenzylaminostyryl)-4-benzyl-5-(4-N,N-dibenzylaminophenyl)pyrazoline  
 (94) 1-[pyridyl-(3)]-3-(4-N-ethyl-N-propylaminostyryl)-4-chloro-5-(4-N-ethyl-N-propylaminophenyl)pyrazoline  
 (95) 1-[pyridyl-(3)]-3-(4-N,N-diethylaminostyryl)-4-benzyl-5-(4-N,N-dibenzylaminophenyl)pyrazoline  
 (96) 1-[pyridyl-(3)]-3-(4-morpholinostyryl)-4-benzyl-5-(4-morpholinophenyl)pyrazoline  
 (97) 1-[pyridyl-(3)]-3-(4-piperidinostyryl)-4-benzyl-5-(4-piperidinophenyl)pyrazoline  
 (98) 1-[pyridyl-(3)]-3-(4-pyrrolidinostyryl)-4-benzyl-5-(4-pyrrolidinophenyl)pyrazoline  
 (99) 1-[pyridyl-(3)]-3-(4-methoxystyryl)-4-benzyl-5-(4-methoxyphenyl)pyrazoline  
 (100) 1-[pyridyl-(3)]-3-(4-ethoxystyryl)-4-benzyl-5-(4-ethoxyphenyl)pyrazoline  
 (101) 1-[pyridyl-(3)]-3-(4-N,N-diethylaminostyryl)-4-benzyl-5-(4-methoxyphenyl)pyrazoline  
 (102) 1-[pyridyl-(3)]-4-benzyl-5,5-diphenyl-3-(4-N,N-diethylaminostyryl)pyrazoline  
 (103) 1-[pyridyl-(3)]-4-benzyl-3,5-di-(4-N,N-diethylaminophenyl)pyrazoline  
 (104) 1-[pyridyl-(3)]-4-benzyl-3,5-di-(4-N,N-dibenzylaminophenyl)pyrazoline

-continued

- 5 (105) 1-[pyridyl-(3)]-4-benzyl-3,5-di-(4-morpholinophenyl)pyrazoline  
 (106) 1-[pyridyl-(3)]-3-(4-N,N-dimethylaminostyryl)-4-phenyl-5-(4-N,N-diethylaminophenyl)pyrazoline  
 (107) 1-[pyridyl-(3)]-3-(4-N,N-diethylaminostyryl)-4-phenyl-5-(4-N,N-diethylaminophenyl)pyrazoline  
 (108) 1-[pyridyl-(3)]-3-(4-N,N-diethylaminostyryl)-4-(4-methylphenyl)-5-(4-N,N-dibenzylaminophenyl)pyrazoline  
 10 (109) 1-[pyridyl-(3)]-3-(4-N,N-diethylaminostyryl)-4-(3-methoxyphenyl)-5-(4-N,N-dibenzylaminophenyl)pyrazoline  
 (110) 1-[pyridyl-(3)]-3-(4-morpholinostyryl)-4-phenyl-5-(4-morpholinophenyl)pyrazoline  
 (111) 1-[pyridyl-(3)]-3-(4-piperidinostyryl)-4-phenyl-5-(4-piperidinophenyl)pyrazoline  
 15 (112) 1-[pyridyl-(3)]-3-(4-pyrrolidinostyryl)-4-phenyl-5-(4-pyrrolidinophenyl)pyrazoline  
 (113) 1-[6-methoxy-pyridyl-(2)]-3-(4-N,N-dimethylaminostyryl)-4-methyl-5-(4-N,N-dimethylaminophenyl)pyrazoline  
 20 (114) 1-[6-methoxy-pyridyl-(2)]-3-(4-N,N-diethylaminostyryl)-4-methyl-5-(4-N,N-diethylaminophenyl)pyrazoline  
 (115) 1-[6-methoxy-pyridyl-(2)]-3-(4-N,N-diethylaminostyryl)-4-ethyl-5-(4-N,N-dibenzylaminophenyl)pyrazoline  
 25 (116) 1-[6-methoxy-pyridyl-(2)]-3-(4-N-ethyl-N-propylaminostyryl)-4-phenyl-5-(4-N-ethyl-N-propylaminophenyl)pyrazoline  
 (117) 1-[6-methoxy-pyridyl-(2)]-3-(4-N,N-diethylaminostyryl)-4-chloro-5-(4-N,N-dibenzylaminophenyl)pyrazoline  
 30 (118) 1-[6-methoxy-pyridyl-(2)]-3-(4-morpholinostyryl)-4-methyl-5-(4-morpholinophenyl)pyrazoline  
 (119) 1-[6-methoxy-pyridyl-(2)]-3-(4-piperidinostyryl)-4-methyl-5-(4-piperidinophenyl)pyrazoline  
 (120) 1-[6-methoxy-pyridyl-(2)]-3-(4-pyrrolidinostyryl)-4-methyl-5-(4-pyrrolidinophenyl)pyrazoline  
 (121) 1-[6-methoxy-pyridyl-(2)]-3-(4-methoxyphenyl)-4-methyl-5-(4-methoxyphenyl)pyrazoline  
 35 (122) 1-[6-methoxy-pyridyl-(2)]-3-(4-ethoxystyryl)-4-methyl-5-(4-ethoxyphenyl)pyrazoline  
 (123) 1-[6-methoxy-pyridyl-(2)]-3-(4-N,N-diethylaminostyryl)-4-methyl-5-(4-methoxyphenyl)pyrazoline  
 (124) 1-[quinolyl-(2)]-3-(4-N,N-dimethylaminostyryl)-4-methyl-5-(4-N,N-dimethylaminophenyl)pyrazoline  
 40 (125) 1-[quinolyl-(2)]-3-(4-N,N-diethylaminostyryl)-4-methyl-5-(4-N,N-diethylaminophenyl)pyrazoline  
 (126) 1-[quinolyl-(2)]-3-(4-N,N-dibenzylaminostyryl)-4-ethyl-5-(4-N,N-dibenzylaminophenyl)pyrazoline  
 45 (127) 1-[quinolyl-(2)]-3-(4-N-ethyl-N-propylaminostyryl)-4-methyl-5-(4-N-ethyl-N-propylaminophenyl)pyrazoline  
 (128) 1-[quinolyl-(2)]-3-(4-N,N-diethylaminostyryl)-4-methyl-5-(4-N,N-dibenzylaminophenyl)pyrazoline  
 (129) 1-[quinolyl-(2)]-3-(4-morpholinostyryl)-4-methyl-5-(4-morpholinophenyl)pyrazoline  
 50 (130) 1-[quinolyl-(2)]-3-(4-piperidinostyryl)-4-methyl-5-(4-piperidinophenyl)pyrazoline  
 (131) 1-[quinolyl-(2)]-3-(4-pyrrolidinostyryl)-4-methyl-5-(4-pyrrolidinophenyl)pyrazoline  
 (132) 1-[quinolyl-(2)]-3-(4-methoxystyryl)-4-methyl-5-(4-methoxyphenyl)pyrazoline  
 55 (133) 1-[quinolyl-(2)]-3-(4-ethoxystyryl)-4-methyl-5-(4-ethoxyphenyl)pyrazoline  
 (134) 1-[quinolyl-(2)]-3-(4-N,N-dimethylaminostyryl)-4-methyl-5-(4-methoxyphenyl)pyrazoline  
 (135) 1-[lepidyl-(2)]-3-(4-N,N-dimethylaminostyryl)-4-methyl-5-(4-N,N-dimethylaminophenyl)pyrazoline  
 60 (136) 1-[lepidyl-(2)]-3-(4-N,N-diethylaminostyryl)-4-methyl-5-(4-N,N-diethylaminophenyl)pyrazoline  
 (137) 1-[lepidyl-(2)]-3-(4-N,N-dibenzylaminostyryl)-4-propyl-5-(4-N,N-dibenzylaminophenyl)pyrazoline  
 (138) 1-[lepidyl-(2)]-3-(4-N-ethyl-N-propylaminostyryl)-4-(4-methylbenzyl)-5-(4-N-ethyl-N-propylaminophenyl)pyrazoline  
 65 (139) 1-[lepidyl-(2)]-3-(4-N,N-diethylaminostyryl)-4-methyl-5-(4-N,N-dibenzylaminophenyl)pyrazoline  
 (140) 1-[lepidyl-(2)]-3-(4-morpholinostyryl)-

-continued

- (141) 1-[lepidyl-(2)]-3-(4-piperidinostyryl)-4-methyl-5-(4-piperidinophenyl)pyrazoline
- (142) 1-[lepidyl-(2)]-3-(4-pyrrolidinostyryl)-4-methyl-5-(4-pyrrolidinophenyl)pyrazoline
- (143) 1-[lepidyl-(2)]-3-(4-methoxystyryl)-4-methyl-5-(4-methoxyphenyl)pyrazoline
- (144) 1-[lepidyl-(2)]-3-(4-ethoxystyryl)-4-methyl-5-(4-ethoxyphenyl)pyrazoline
- (145) 1-[lepidyl-(2)]-3-(4-N,N-diethylamino-styryl)-4-methyl-5-(4-methoxyphenyl)pyrazoline
- (146) 1-[pyridyl-(2)]-3-(4-N,N-dimethylamino-styryl)-4-methyl-5-(4-N,N-dimethylaminophenyl)pyrazoline
- (147) 1-[pyridyl-(2)]-3-(4-N,N-diethylamino-styryl)-4-methyl-5-(4-N,N-diethylaminophenyl)pyrazoline
- (148) 1-[pyridyl-(2)]-3-(4-N,N-dibenzylamino-styryl)-4-methyl-5-(4-N,N-dibenzylaminophenyl)pyrazoline
- (149) 1-[pyridyl-(2)]-3-(4-N-ethyl-N-propyl-aminostyryl)-4-methyl-5-(4-N-ethyl-N-propylaminophenyl)pyrazoline
- (150) 1-[pyridyl-(2)]-3-(4-N,N-diethylamino-styryl)-4-methyl-5-(4-N,N-dibenzylaminophenyl)pyrazoline
- (151) 1-[pyridyl-(2)]-3-(4-morpholinostyryl)-4-methyl-5-(4-morpholinophenyl)pyrazoline
- (152) 1-[pyridyl-(2)]-3-(4-piperidinostyryl)-4-methyl-5-(4-piperidinophenyl)pyrazoline
- (153) 1-[pyridyl-(2)]-3-(4-pyrrolidinostyryl)-4-methyl-5-(4-pyrrolidinophenyl)pyrazoline
- (154) 1-[pyridyl-(2)]-3-(4-methoxystyryl)-4-methyl-5-(4-methoxyphenyl)pyrazoline
- (155) 1-[pyridyl-(2)]-3-(4-ethoxystyryl)-4-methyl-5-(4-ethoxyphenyl)pyrazoline
- (156) 1-[pyridyl-(2)]-3-(4-N,N-diethylamino-styryl)-4-methyl-5-(4-methoxyphenyl)pyrazoline
- (157) 1-[carbazolyl-(3)]-3-(4-N,N-dimethyl-aminostyryl)-4-methyl-5-(4-N,N-dimethylaminophenyl)pyrazoline
- (158) 1-[carbazolyl-(3)]-3-(4-N,N-diethylamino-styryl)-4-methyl-5-(4-N,N-diethylaminophenyl)pyrazoline
- (159) 1-[carbazolyl-(3)]-3-(4-N,N-diethyl-aminostyryl)-4-phenyl-5-(4-N,N-diethylaminophenyl)pyrazoline
- (160) 1-[9-ethyl-carbazolyl-(3)]-3-(4-N,N-diethylaminostyryl)-4-methyl-5-(4-N,N-diethylamino-phenyl)pyrazoline
- (161) 1-[9-ethyl-carbazolyl-(3)]-3-(4-N,N-diethylaminostyryl)-4-benzyl-5-(4-N,N-diethylamino-phenyl)pyrazoline
- (162) 1-[pyridyl-(3)]-3-( $\alpha$ -methyl-4-N,N-diethylaminostyryl)-5-(4-N,N-diethylaminophenyl)pyrazoline
- (163) 1-[pyridyl-(3)]-3-( $\alpha$ -methyl-4-N,N-diethylaminostyryl)-4-methyl-5-(4-N,N-diethylamino-phenyl)pyrazoline
- (164) 1-[lepidyl-(2)]-3-( $\alpha$ -benzyl-4-N,N-diethylaminostyryl)-4-methyl-5-(4-N,N-diethylamino-phenyl)pyrazoline
- 5 (165) 1-[pyridyl-(3)]-3-(4-N,N-dimethylamino-styryl)-5-[furyl-(2)]pyrazoline
- (166) 1-[pyridyl-(3)]-3-(4-N,N-diethylamino-styryl)-5-[furyl-(2)]pyrazoline
- (167) 1-[pyridyl-(3)]-3-(4-N,N-dibenzylamino-styryl)-5-[furyl-(2)]pyrazoline
- (168) 1-[pyridyl-(3)]-3-(4-N,N-dipropylamino-styryl)-5-[furyl-(2)]pyrazoline
- (169) 1-[pyridyl-(3)]-3-(4-N,N-dibutylamino-styryl)-5-[furyl-(2)]pyrazoline
- (170) 1-[pyridyl-(3)]-3-(4-N-ethyl-N-butyl-aminostyryl)-5-[furyl-(2)]pyrazoline
- (171) 1-[pyridyl-(3)]-3-(4-N,N-diphenylamino-styryl)-5-[furyl-(2)]pyrazoline
- (172) 1-[pyridyl-(3)]-3-(4-piperidinostyryl)-5-[furyl-(2)]pyrazoline
- (173) 1-[pyridyl-(3)]-3-(4-pyrrolidinostyryl)-5-[furyl-(2)]pyrazoline
- (174) 1-[pyridyl-(3)]-3-(4-morpholinostyryl)-5-[furyl-(2)]pyrazoline
- (175) 1,5-di-[pyridyl-(3)]-3-(4-N,N-diethylamino-styryl)pyrazoline
- (176) 1,5-di-[pyridyl-(3)]-3-(4-N,N-dibenzylamino-styryl)pyrazoline
- (177) 1,5-di-[pyridyl-(3)]-3-(4-piperidino-styryl)pyrazoline
- (178) 1-[pyridyl-(3)]-3-(4-N,N-diethylamino-styryl)-5-[N-methyl-imidazolyl-(4)]pyrazoline
- (179) 1-[pyridyl-(3)]-3-(4-N,N-dibenzylamino-styryl)-5-[N-methyl-imidazolyl-(4)]pyrazoline
- (180) 1-[pyridyl-(3)]-3-(4-N,N-diethylamino-styryl)-5-[N-3-methoxypropyl-imidazolyl-(4)]pyrazoline
- (181) 1-[pyridyl-(3)]-3-(4-N,N-diethylamino-styryl)-5-[N-ethyl-oxazolyl-(4)]pyrazoline
- (182) 1-[pyridyl-(3)]-3-(4-N,N-diethylamino-styryl)-5-[N-ethyl-carbazolyl-(3)]pyrazoline
- (183) 1-[pyridyl-(3)]-3-(4-N,N-diethylamino-styryl)-5-[N-ethyl-thiazolyl-(4)]pyrazoline
- (184) 1,5-di-[pyridyl-(3)]-3-(4-N,N-diethylamino-styryl)-5-(4-methoxyphenyl)pyrazoline
- 20 (185) 1-[pyridyl-(3)]-3-[8-(3-pyridyl)vinyl]-5-[furyl-(2)]pyrazoline
- (186) 1-[pyridyl-(3)]-3-[8-(2-furyl)vinyl]-5-[furyl-(2)]pyrazoline
- (187) 1-[pyridyl-(3)]-3,5-di-[furyl-(2)]pyrazoline
- (188) 1-[pyridyl-(3)]-3-(4-N,N-diethylamino-styryl)-4-methyl-5-[furyl-(2)]pyrazoline
- (189) 1-[pyridyl-(3)]-3-(4-N,N-diethylamino-styryl)-4-benzyl-5-[furyl-(2)]pyrazoline
- (190) 1-[pyridyl-(3)]-3-(4-N,N-diethylamino-styryl)-4-phenyl-5-[furyl-(2)]pyrazoline
- (191) 1-[pyridyl-(3)]-3-( $\alpha$ -methyl-4-N,N-diethylamino-styryl)-5-[furyl-(2)]pyrazoline
- (192) 1-[pyridyl-(3)]-3-( $\alpha$ -benzyl-4-N,N-diethylamino-styryl)-5-[furyl-(2)]pyrazoline
- (193) 1-[pyridyl-(3)]-3-( $\alpha$ -phenyl-4-N,N-diethylamino-styryl)-5-[furyl-(2)]pyrazoline
- (194) 1-[quinolyl-(2)]-3-(4-N,N-dimethylamino-styryl)-5-[furyl-(2)]pyrazoline
- 25 (195) 1-[quinolyl-(2)]-3-(4-N,N-diethylamino-styryl)-5-[furyl-(2)]pyrazoline
- (196) 1-[quinolyl-(2)]-3-(4-N,N-dibenzylamino-styryl)-5-[furyl-(2)]pyrazoline
- (197) 1-[quinolyl-(2)]-3-(4-N,N-dipropylamino-styryl)-5-[furyl-(2)]pyrazoline
- (198) 1-[quinolyl-(2)]-3-(4-N,N-dibutylamino-styryl)-5-[furyl-(2)]pyrazoline
- (199) 1-[quinolyl-(2)]-3-(4-N-ethyl-N-butylamino-styryl)-5-[furyl-(2)]pyrazoline
- (200) 1-[quinolyl-(2)]-3-(4-N,N-diphenylamino-styryl)-5-[furyl-(2)]pyrazoline
- 30 (201) 1-[quinolyl-(2)]-3-(4-piperidinostyryl)-5-[furyl-(2)]pyrazoline
- (202) 1-[quinolyl-(2)]-3-(4-pyrrolidinostyryl)-5-[furyl-(2)]pyrazoline
- (203) 1-[quinolyl-(2)]-3-(4-morpholinostyryl)-5-[furyl-(2)]pyrazoline
- (204) 1,5-di-[quinolyl-(2)]-3-(4-N,N-diethylamino-styryl)pyrazoline
- (205) 1,5-di-[quinolyl-(2)]-3-(4-N,N-dibenzylamino-styryl)pyrazoline
- (206) 1,5-di-[quinolyl-(2)]-3-(4-piperidino-

These compounds are also readily prepared by known synthetic methods, for instance, by refluxing an unsaturated ketone and a hydrazino compound represented by the following formulae (c) and (d), respectively, in alcohol in the presence of a small amount of acetic acid for several hours.



(n, R<sub>1</sub>, R<sub>2</sub>, R<sub>3</sub>, R<sub>4</sub>, R<sub>5</sub> and X<sub>1</sub> are as defined above)

- 50 (195) 1-[quinolyl-(2)]-3-(4-N,N-diethylamino-styryl)-5-[furyl-(2)]pyrazoline
- (196) 1-[quinolyl-(2)]-3-(4-N,N-dibenzylamino-styryl)-5-[furyl-(2)]pyrazoline
- (197) 1-[quinolyl-(2)]-3-(4-N,N-dipropylamino-styryl)-5-[furyl-(2)]pyrazoline
- (198) 1-[quinolyl-(2)]-3-(4-N,N-dibutylamino-styryl)-5-[furyl-(2)]pyrazoline
- (199) 1-[quinolyl-(2)]-3-(4-N-ethyl-N-butylamino-styryl)-5-[furyl-(2)]pyrazoline
- (200) 1-[quinolyl-(2)]-3-(4-N,N-diphenylamino-styryl)-5-[furyl-(2)]pyrazoline
- 55 (201) 1-[quinolyl-(2)]-3-(4-piperidinostyryl)-5-[furyl-(2)]pyrazoline
- (202) 1-[quinolyl-(2)]-3-(4-pyrrolidinostyryl)-5-[furyl-(2)]pyrazoline
- (203) 1-[quinolyl-(2)]-3-(4-morpholinostyryl)-5-[furyl-(2)]pyrazoline
- (204) 1,5-di-[quinolyl-(2)]-3-(4-N,N-diethylamino-styryl)pyrazoline
- (205) 1,5-di-[quinolyl-(2)]-3-(4-N,N-dibenzylamino-styryl)pyrazoline
- (206) 1,5-di-[quinolyl-(2)]-3-(4-piperidino-

-continued

- styryl)pyrazoline  
 (207) 1-[quinolyl-(2)]-3-(4-N,N-diethylamino-styryl)-5-[N-methyl-imidazolyl-(4)]pyrazoline  
 (208) 1-[quinolyl-(2)]-3-(4-N,N-dibenzylamino-styryl)-5-[N-methyl-imidazolyl-(4)]pyrazoline  
 (209) 1-[quinolyl-(2)]-3-(4-N,N-diethylamino-styryl)-5-[N-3-methoxypropyl-imidazolyl-(4)]pyrazoline  
 (210) 1-[quinolyl-(2)]-3-(4-N,N-diethylamino-styryl)-5-[N-ethyl-oxazolyl-(4)]pyrazoline  
 (211) 1-[quinolyl-(2)]-3-(4-N,N-diethylamino-styryl)-5-[N-ethyl-carbazolyl-(3)]pyrazoline  
 (212) 1-[quinolyl-(2)]-3-(4-N,N-diethylamino-styryl)-5-[N-ethyl-thiazolyl-(4)]pyrazoline  
 (213) 1,5-di-[quinolyl-(2)]-3-(4-N,N-diethylaminophenyl)pyrazoline  
 (214) 1-[quinolyl-(2)]-3-[ $\beta$ -(3-pyridyl)vinyl]-5-[furyl-(2)]pyrazoline  
 (215) 1-[quinolyl-(2)]-3-[ $\beta$ -(2-furyl)vinyl]-5-[furyl-(2)]pyrazoline  
 (216) 1-[quinolyl-(2)]-3,5-di-[furyl-(2)]-pyrazoline  
 (217) 1-[quinolyl-(2)]-3-(4-N,N-diethylamino-styryl)-4-methyl-5-[furyl-(2)]pyrazoline  
 (218) 1-[quinolyl-(2)]-3-(4-N,N-diethylamino-styryl)-4-benzyl-5-[furyl-(2)]pyrazoline  
 (219) 1-[quinolyl-(2)]-3-(4-N,N-diethylamino-styryl)-4-phenyl-5-[furyl-(2)]pyrazoline  
 (220) 1-[quinolyl-(2)]-3-( $\alpha$ -methyl-4-N,N-diethylaminostyryl)-5-[furyl-(2)]pyrazoline  
 (221) 1-[quinolyl-(2)]-3-( $\alpha$ -benzyl-4-N,N-diethylaminostyryl)-5-[furyl-(2)]pyrazoline  
 (222) 1-[quinolyl-(2)]-3-( $\alpha$ -phenyl-4-N,N-diethylaminostyryl)-5-[furyl-(2)]pyrazoline  
 (223) 1-[lepidyl-(2)]-3-(4-N,N-dimethylamino-styryl)-5-[furyl-(2)]pyrazoline  
 (224) 1-[lepidyl-(2)]-3-(4-N,N-diethylamino-styryl)-5-[furyl-(2)]pyrazoline  
 (225) 1-[lepidyl-(2)]-3-(4-N,N-dibenzylamino-styryl)-5-[furyl-(2)]pyrazoline  
 (226) 1-[lepidyl-(2)]-3-(4-N,N-dipropylamino-styryl)-5-[furyl-(2)]pyrazoline  
 (227) 1-[lepidyl-(2)]-3-(4-N,N-dibutylamino-styryl)-5-[furyl-(2)]pyrazoline  
 (228) 1-[lepidyl-(2)]-3-(4-N-ethyl-N-butylaminostyryl)-5-[furyl-(2)]pyrazoline  
 (229) 1-[lepidyl-(2)]-3-(4-N,N-diphenylamino-styryl)-5-[furyl-(2)]pyrazoline  
 (230) 1-[lepidyl-(2)]-3-(4-piperidinostyryl)-5-[furyl-(2)]pyrazoline  
 (231) 1-[lepidyl-(2)]-3-(4-pyrrolidinostyryl)-5-[furyl-(2)]pyrazoline  
 (232) 1-[lepidyl-(2)]-3-(4-morpholinostyryl)-5-[furyl-(2)]pyrazoline  
 (233) 1,5-di-[lepidyl-(2)]-3-(4-N,N-diethylamino-styryl)pyrazoline  
 (234) 1,5-di-[lepidyl-(2)]-3-(4-N,N-dibenzylamino-styryl)pyrazoline  
 (235) 1,5-di-[lepidyl-(2)]-3-(4-piperidinostyryl)-pyrazoline  
 (236) 1-[lepidyl-(2)]-3-(4-N,N-diethylamino-styryl)-5-[N-methyl-imidazolyl-(4)]pyrazoline  
 (237) 1-[lepidyl-(2)]-3-(4-N,N-dibenzylamino-styryl)-5-[N-methyl-imidazolyl-(4)]pyrazoline  
 (238) 1-[lepidyl-(2)]-3-(4-N,N-diethylamino-styryl)-5-[N-3-methoxypropyl-imidazolyl-(4)]pyrazoline  
 (239) 1-[lepidyl-(2)]-3-(4-N,N-diethylamino-styryl)-5-[N-ethyl-oxazolyl-(4)]pyrazoline  
 (240) 1-[lepidyl-(2)]-3-(4-N,N-diethylamino-styryl)-5-[N-ethyl-carbazolyl-(3)]pyrazoline  
 (241) 1-[lepidyl-(2)]-3-(4-N,N-diethylamino-styryl)-5-[N-ethyl-thiazolyl-(4)]pyrazoline  
 (242) 1,5-di-[lepidyl-(2)]-3-(4-N,N-diethylaminophenyl)pyrazoline  
 (243) 1-[lepidyl-(2)]-3-[ $\beta$ -(3-pyridyl)vinyl]-5-[furyl-(2)]pyrazoline  
 (244) 1-[lepidyl-(2)]-3-[ $\beta$ -(2-furyl)vinyl]-5-[furyl-(2)]pyrazoline  
 (245) 1-[lepidyl-(2)]-3,5-di-[furyl-(2)]-pyrazoline  
 (246) 1-[lepidyl-(2)]-3-(4-N,N-diethylamino-styryl)-4-methyl-5-[furyl-(2)]pyrazoline  
 (247) 1-[lepidyl-(2)]-3-(4-N,N-diethylamino-

-continued

- styryl)-4-benzyl-5-[furyl-(2)]pyrazoline  
 (248) 1-[lepidyl-(2)]-3-(4-N,N-diethylamino-styryl)-4-phenyl-5-[furyl-(2)]pyrazoline  
 5 (249) 1-[lepidyl-(2)]-3-( $\alpha$ -methyl-4-N,N-diethylaminostyryl)-5-[furyl-(2)]pyrazoline  
 (250) 1-[lepidyl-(2)]-3-( $\alpha$ -benzyl-4-N,N-diethylaminostyryl)-5-[furyl-(2)]pyrazoline  
 (251) 1-[lepidyl-(2)]-3-( $\alpha$ -phenyl-4-N,N-diethylaminostyryl)-5-[furyl-(2)]pyrazoline  
 10 (252) 1-[pyridyl-(2)]-3-(4-N,N-dimethylamino-styryl)-5-[furyl-(2)]pyrazoline  
 (253) 1-[pyridyl-(2)]-3-(4-N,N-diethylamino-styryl)-5-[furyl-(2)]pyrazoline  
 (254) 1-[pyridyl-(2)]-3-(4-N,N-dibenzylamino-styryl)-5-[furyl-(2)]pyrazoline  
 15 (255) 1-[pyridyl-(2)]-3-(4-N,N-dipropylamino-styryl)-5-[furyl-(2)]pyrazoline  
 (256) 1-[6-methoxy-pyridyl-(2)]-3-(4-N,N-dibutylaminostyryl)-5-[furyl-(2)]pyrazoline  
 (257) 1-[pyridyl-(2)]-3-(4-N-ethyl-N-butylaminostyryl)-5-[furyl-(2)]pyrazoline  
 20 (258) 1-[pyridyl-(2)]-3-(4-N,N-diphenylamino-styryl)-5-[furyl-(2)]pyrazoline  
 (259) 1-[pyridyl-(2)]-3-(4-piperidinostyryl)-5-[furyl-(2)]pyrazoline  
 (260) 1-[pyridyl-(2)]-3-(4-pyrrolidinostyryl)-5-[furyl-(2)]pyrazoline  
 (261) 1-[pyridyl-(2)]-3-(4-morpholinostyryl)-5-[furyl-(2)]pyrazoline  
 (262) 1,5-di-[pyridyl-(2)]-3-(4-N,N-diethylamino-styryl)pyrazoline  
 (263) 1,5-di-[pyridyl-(2)]-3-(4-N,N-dibenzylamino-styryl)pyrazoline  
 30 (264) 1,5-di-[pyridyl-(2)]-3-(4-piperidino-styryl)pyrazoline  
 (265) 1-[pyridyl-(2)]-3-(4-N,N-diethylamino-styryl)-5-[N-methyl-imidazolyl-(4)]pyrazoline  
 (266) 1-[pyridyl-(2)]-3-(4-N,N-dibenzylamino-styryl)-5-[N-methyl-imidazolyl-(4)]pyrazoline  
 (267) 1-[pyridyl-(2)]-3-(4-N,N-diethylamino-styryl)-5-[N-3-methoxypropyl-imidazolyl-(4)]pyrazoline  
 35 (268) 1-[pyridyl-(2)]-3-(4-N,N-diethylamino-styryl)-5-[N-ethyl-oxazolyl-(4)]pyrazoline  
 (269) 1-[pyridyl-(2)]-3-(4-N,N-diethylamino-styryl)-5-[N-ethyl-carbazolyl-(3)]pyrazoline  
 (270) 1-[pyridyl-(2)]-3-(4-N,N-diethylamino-styryl)-5-[N-ethyl-thiazolyl-(4)]pyrazoline  
 40 (271) 1,5-di-[pyridyl-(2)]-3-(4-N,N-diethylamino-phenyl)pyrazoline  
 (272) 1-[pyridyl-(2)]-3-[ $\beta$ -(3-pyridyl)vinyl]-5-[furyl-(2)]pyrazoline  
 (273) 1-[pyridyl-(2)]-3-[ $\beta$ -(2-furyl)vinyl]-5-[furyl-(2)]pyrazoline  
 45 (274) 1-[pyridyl-(2)]-3,5-di-[furyl-(2)]-pyrazoline  
 (275) 1-[pyridyl-(2)]-3-(4-N,N-diethylamino-styryl)-4-methyl-5-[furyl-(2)]pyrazoline  
 (276) 1-[pyridyl-(2)]-3-(4-N,N-diethylamino-styryl)-4-benzyl-5-[furyl-(2)]pyrazoline  
 50 (277) 1-[pyridyl-(2)]-3-(4-N,N-diethylamino-styryl)-4-phenyl-5-[furyl-(2)]pyrazoline  
 (278) 1-[pyridyl-(2)]-3-( $\alpha$ -methyl-4-N,N-diethylaminostyryl)-5-[furyl-(2)]pyrazoline  
 (279) 1-[pyridyl-(2)]-3-( $\alpha$ -benzyl-4-N,N-diethylaminostyryl)-5-[furyl-(2)]pyrazoline  
 55 (280) 1-[pyridyl-(2)]-3-( $\alpha$ -phenyl-4-N,N-diethylaminostyryl)-5-[furyl-(2)]pyrazoline  
 (281) 1-[pyridyl-(2)]-3-(4-methoxystyryl)-5-[furyl-(2)]pyrazoline  
 (282) 1-[quinolyl-(2)]-3-(4-methoxystyryl)-5-[furyl-(2)]pyrazoline  
 60 (283) 1-[N-ethyl-carbazolyl-(3)]-3-(4-N,N-diethylaminostyryl)-5-[furyl-(2)]pyrazoline

These compounds are also readily prepared by known synthetic methods, for instance, by refluxing an unsaturated ketone and a hydrazino compound represented by the following formulae (e) and (f), respectively, in alcohol in the presence of a small amount of acetic acid for several hours.

## Formula

(R<sub>1</sub>, R<sub>2</sub>, R<sub>4</sub>, R<sub>5</sub>, X<sub>1</sub>, and n are as defined above)

- 284) 1-[pyridyl-(3)]-3-[ $\beta$ -(2-furyl)vinyl]-5-(4-N,N-diethylaminophenyl)pyrazoline
- 285) 1-[pyridyl-(3)]-3-[ $\beta$ -(2-furyl)vinyl]-5-(4-N,N-diethylaminophenyl)pyrazoline
- 286) 1-[pyridyl-(3)]-3-[ $\beta$ -(2-furyl)vinyl]-5-(4-N,N-dibenzylaminophenyl)pyrazoline
- 287) 1-[pyridyl-(3)]-3-[ $\beta$ -(2-furyl)vinyl]-5-(4-N-ethyl-N-propylaminophenyl)pyrazoline
- 288) 1-[pyridyl-(3)]-3-[ $\beta$ -(2-furyl)vinyl]-5-(4-N,N-dibutylaminophenyl)pyrazoline
- 289) 1-[pyridyl-(3)]-3-[ $\beta$ -(2-furyl)vinyl]-4-methyl-5-(4-N,N-diethylaminophenyl)pyrazoline
- 290) 1-[pyridyl-(3)]-3-[ $\beta$ -(2-furyl)vinyl]-4-benzyl-5-(4-N,N-diethylaminophenyl)pyrazoline
- 291) 1-[pyridyl-(3)]-3-[ $\beta$ -(2-furyl)vinyl]-4-phenyl-5-(4-N,N-diethylaminophenyl)pyrazoline
- 292) 1-[pyridyl-(3)]-3-[ $\alpha$ -methyl- $\beta$ -(2-furyl)vinyl]-5-(4-N,N-diethylaminophenyl)pyrazoline
- 293) 1-[pyridyl-(3)]-3-[ $\alpha$ -benzyl- $\beta$ -(2-furyl)vinyl]-5-(4-N,N-diethylaminophenyl)pyrazoline
- 294) 1-[pyridyl-(3)]-3-[ $\alpha$ -phenyl- $\beta$ -(2-furyl)vinyl]-5-(4-N,N-diethylaminophenyl)pyrazoline
- 295) 1-[pyridyl-(3)]-3-[furyl-(2)]-5-(4-N,N-diethylaminophenyl)pyrazoline
- 296) 1-[pyridyl-(3)]-3-[ $\beta$ -(N-ethyl-3-carbazolyl)vinyl]-5-(4-N,N-diethylaminophenyl)pyrazoline
- 297) 1-[pyridyl-(3)]-3-[ $\beta$ -(N-methyl-4-imidazolyl)vinyl]-5-(4-N,N-diethylaminophenyl)pyrazoline
- 298) 1-[pyridyl-(3)]-3-[ $\beta$ -(N-ethyl-4-imidazolyl)vinyl]-5-(4-N,N-diethylaminophenyl)pyrazoline
- 299) 1-[pyridyl-(3)]-3-[ $\beta$ -(N-ethyl-4-oxazolyl)vinyl]-5-(4-N,N-diethylaminophenyl)pyrazoline
- 300) 1-[pyridyl-(3)]-3-[ $\beta$ -(N-ethyl-4-thiazolyl)vinyl]-5-(4-N,N-diethylaminophenyl)pyrazoline
- 301) 1,3-di-[pyridyl-(3)]-5-(4-N,N-diethylaminophenyl)pyrazoline
- 302) 1-[pyridyl-(3)]-3-[ $\beta$ -(N-ethyl-3-carbazolyl)vinyl]-5-(4-methoxyphenyl)pyrazoline
- 303) 1-[pyridyl-(3)]-3-[ $\alpha$ -methyl- $\beta$ -(2-furyl)vinyl]-4-methyl-5-(4-methoxyphenyl)pyrazoline
- 304) 1-[quinolyl-(2)]-3-[ $\beta$ -(2-furyl)vinyl]-5-(4-N,N-dimethylaminophenyl)pyrazoline
- 305) 1-[quinolyl-(2)]-3-[ $\beta$ -(2-furyl)vinyl]-5-(4-N,N-diethylaminophenyl)pyrazoline
- 306) 1-[quinolyl-(2)]-3-[ $\beta$ -(2-furyl)vinyl]-5-(4-N,N-dibenzylaminophenyl)pyrazoline
- 307) 1-[quinolyl-(2)]-3-[ $\beta$ -(2-furyl)vinyl]-5-(4-N-ethyl-N-propylaminophenyl)pyrazoline
- 308) 1-[quinolyl-(2)]-3-[ $\beta$ -(2-furyl)vinyl]-5-(4-N,N-dibutylaminophenyl)pyrazoline
- 309) 1-[quinolyl-(2)]-3-[ $\beta$ -(2-furyl)vinyl]-4-methyl-5-(4-N,N-diethylaminophenyl)pyrazoline
- 310) 1-[quinolyl-(2)]-3-[ $\beta$ -(2-furyl)vinyl]-4-benzyl-5-(4-N,N-diethylaminophenyl)pyrazoline
- 311) 1-[quinolyl-(2)]-3-[ $\beta$ -(2-furyl)vinyl]-4-phenyl-5-(4-N,N-diethylaminophenyl)pyrazoline
- 312) 1-[quinolyl-(2)]-3-[ $\alpha$ -methyl- $\beta$ -(2-furyl)vinyl]-5-(4-N,N-diethylaminophenyl)pyrazoline
- 313) 1-[quinolyl-(2)]-3-[ $\alpha$ -benzyl- $\beta$ -(2-furyl)vinyl]-5-(4-N,N-diethylaminophenyl)pyrazoline
- 314) 1-[quinolyl-(2)]-3-[ $\alpha$ -phenyl- $\beta$ -(2-furyl)vinyl]-5-(4-N,N-diethylaminophenyl)pyrazoline
- 315) 1-[quinolyl-(2)]-3-[furyl-(2)]-5-(4-N,N-diethylaminophenyl)pyrazoline
- 316) 1-[quinolyl-(2)]-3-[ $\beta$ -(N-ethyl-3-carbazolyl)vinyl]-5-(4-N,N-diethylaminophenyl)pyrazoline
- 317) 1-[quinolyl-(2)]-3-[ $\beta$ -(N-methyl-4-imidazolyl)vinyl]-5-(4-N,N-diethylaminophenyl)pyrazoline

-continued

- (318) 1-[quinolyl-(2)]-3-[ $\beta$ -(N-ethyl-4-imidazolyl)vinyl]-5-(4-N,N-diethylaminophenyl)pyrazoline
- 5 (319) 1-[quinolyl-(2)]-3-[ $\beta$ -(N-ethyl-4-oxazolyl)vinyl]-5-(4-N,N-diethylaminophenyl)pyrazoline
- (320) 1-[quinolyl-(2)]-3-[ $\beta$ -(N-ethyl-4-thiazolyl)vinyl]-5-(4-N,N-diethylaminophenyl)pyrazoline
- 10 (321) 1,3-di-[quinolyl-(2)]-5-(4-N,N-diethylaminophenyl)pyrazoline
- (322) 1-[quinolyl-(2)]-3-[ $\beta$ -(N-ethyl-3-carbazolyl)vinyl]-5-(4-methoxyphenyl)pyrazoline
- 15 (324) 1-[lepidyl-(2)]-3-[ $\beta$ -(2-furyl)vinyl]-5-(4-N,N-dimethylaminophenyl)pyrazoline
- (325) 1-[lepidyl-(2)]-3-[ $\beta$ -(2-furyl)vinyl]-5-(4-N,N-diethylaminophenyl)pyrazoline
- (326) 1-[lepidyl-(2)]-3-[ $\beta$ -(2-furyl)vinyl]-5-(4-N,N-dibenzylaminophenyl)pyrazoline
- 20 (327) 1-[lepidyl-(2)]-3-[ $\beta$ -(2-furyl)vinyl]-5-(4-N-ethyl-N-propylaminophenyl)pyrazoline
- (328) 1-[lepidyl-(2)]-3-[ $\beta$ -(2-furyl)vinyl]-5-(4-N,N-dibutylaminophenyl)pyrazoline
- (329) 1-[lepidyl-(2)]-3-[ $\beta$ -(2-furyl)vinyl]-4-methyl-5-(4-N,N-diethylaminophenyl)pyrazoline
- 25 (330) 1-[lepidyl-(2)]-3-[ $\beta$ -(2-furyl)vinyl]-4-benzyl-5-(4-N,N-diethylaminophenyl)pyrazoline
- (331) 1-[lepidyl-(2)]-3-[ $\beta$ -(2-furyl)vinyl]-4-phenyl-5-(4-N,N-diethylaminophenyl)pyrazoline
- (332) 1-[lepidyl-(2)]-3-[ $\alpha$ -methyl- $\beta$ -(2-furyl)vinyl]-5-(4-N,N-diethylaminophenyl)pyrazoline
- 30 (333) 1-[lepidyl-(2)]-3-[ $\alpha$ -benzyl- $\beta$ -(2-furyl)vinyl]-5-(4-N,N-diethylaminophenyl)pyrazoline
- (334) 1-[lepidyl-(2)]-3-[ $\alpha$ -phenyl- $\beta$ -(2-furyl)vinyl]-5-(4-N,N-diethylaminophenyl)pyrazoline
- 35 (335) 1-[lepidyl-(2)]-3-[furyl-(2)]-5-(4-N,N-diethylaminophenyl)pyrazoline
- (336) 1-[lepidyl-(2)]-3-[ $\beta$ -(N-ethyl-3-carbazolyl)vinyl]-5-(4-N,N-diethylaminophenyl)pyrazoline
- (337) 1-[lepidyl-(2)]-3-[ $\beta$ -(N-methyl-4-imidazolyl)vinyl]-5-(4-N,N-diethylaminophenyl)pyrazoline
- 40 (338) 1-[lepidyl-(2)]-3-[ $\beta$ -(N-ethyl-4-imidazolyl)vinyl]-5-(4-N,N-diethylaminophenyl)pyrazoline
- (339) 1-[lepidyl-(2)]-3-[ $\beta$ -(N-ethyl-4-oxazolyl)vinyl]-5-(4-N,N-diethylaminophenyl)pyrazoline
- 45 (340) 1-[lepidyl-(2)]-3-[ $\beta$ -(N-ethyl-4-thiazolyl)vinyl]-5-(4-N,N-diethylaminophenyl)pyrazoline
- (341) 1,3-di-[lepidyl-(2)]-5-(4-N,N-diethylaminophenyl)pyrazoline
- 50 (342) 1-[lepidyl-(2)]-3-[ $\beta$ -(N-ethyl-3-carbazolyl)vinyl]-5-(4-methoxyphenyl)pyrazoline
- (343) 1-[lepidyl-(2)]-3-[ $\alpha$ -methyl- $\beta$ -(2-furyl)vinyl]-4-methyl-5-(4-methoxyphenyl)pyrazoline
- (344) 1-[6-methoxy-pyridyl-(2)]-3-[ $\beta$ -(2-furyl)vinyl]-5-(4-N,N-dimethylaminophenyl)pyrazoline
- (345) 1-[6-methoxy-pyridyl-(2)]-3-[ $\beta$ -(2-furyl)vinyl]-5-(4-N,N-diethylaminophenyl)pyrazoline
- (346) 1-[pyridyl-(2)]-3-[ $\beta$ -(2-furyl)vinyl]-5-(4-N,N-dibenzylaminophenyl)pyrazoline
- 60 (347) 1-[pyridyl-(2)]-3-[ $\beta$ -(2-furyl)vinyl]-5-(4-N-ethyl-N-propylaminophenyl)pyrazoline
- (348) 1-[pyridyl-(2)]-3-[ $\beta$ -(2-furyl)vinyl]-5-(4-N,N-dibutylaminophenyl)pyrazoline
- (349) 1-[pyridyl-(2)]-3-[ $\beta$ -(2-furyl)vinyl]-4-methyl-5-(4-N,N-diethylaminophenyl)pyrazoline
- 65 (350) 1-[pyridyl-(2)]-3-[ $\beta$ -(2-furyl)vinyl]-4-benzyl-5-(4-N,N-diethylaminophenyl)pyrazoline
- (351) 1-[pyridyl-(2)]-3-[ $\beta$ -(2-furyl)vinyl]-4-phenyl-5-(4-N,N-diethylaminophenyl)pyrazoline
- (352) 1-[pyridyl-(2)]-3-[ $\alpha$ -methyl- $\beta$ -(2-furyl)vinyl]-5-(4-N,N-diethylaminophenyl)pyrazoline

-continued

- (2-furyl)vinyl]-5-(4-N,N-diethylaminophenyl)-pyrazoline

(353) 1-[pyridyl-(2)]-3-[ $\alpha$ -benzyl- $\beta$ -(2-furyl)vinyl]-5-(4-N,N-diethylaminophenyl)-pyrazoline

(354) 1-[pyridyl-(2)]-3-[ $\alpha$ -phenyl- $\beta$ -(2-furyl)vinyl]-5-(4-N,N-diethylaminophenyl)-pyrazoline

(355) 1-[pyridyl-(2)]-3-[furyl-(2)]-5-(4-N,N-diethylaminophenyl)pyrazoline

(356) 1-[pyridyl-(2)]-3-[ $\beta$ -(N-ethyl-3-carbazolyl)vinyl]-5-(4-N,N-diethylaminophenyl)-pyrazoline

(357) 1-[pyridyl-(2)]-3-[ $\beta$ -(N-methyl-4-imidazolyl)vinyl]-5-(4-N,N-diethylaminophenyl)-pyrazoline

(358) 1-[pyridyl-(2)]-3-[ $\beta$ -(N-ethyl-4-imidazolyl)vinyl]-5-(4-N,N-diethylaminophenyl)-pyrazoline

(359) 1-[pyridyl-(2)]-3-[ $\beta$ -(N-ethyl-4-oxazolyl)vinyl]-5-(4-N,N-diethylaminophenyl)-pyrazoline

(360) 1-[pyridyl-(2)]-3-[ $\beta$ -(N-ethyl-4-thiazolyl)vinyl]-5-(4-N,N-diethylaminophenyl)-pyrazoline

(361) 1,3-di-[pyridyl-(2)]-5-(4-N,N-diethylaminophenyl)pyrazoline

(362) 1-[pyridyl-(2)]-3-[ $\beta$ -(N-ethyl-3-carbazolyl)vinyl]-5-(4-methoxyphenyl)pyrazoline

(363) 1-[pyridyl-(2)]-3-[ $\alpha$ -methyl- $\beta$ -(2-furyl)vinyl]-4-methyl-5-(4-methoxyphenyl)-pyrazoline

(364) 1-[N-ethyl-carbazolyl-(3)]-3-[ $\beta$ -(2-furyl)vinyl]-5-(4-N,N-diethylaminophenyl)-pyrazoline

(365) 1-[pyridyl-(3)]-3-(4-methoxystyryl)-5-(4-N,N-dimethylaminophenyl)pyrazoline

(366) 1-[pyridyl-(3)]-3-(4-methoxystyryl)-5-(4-N,N-diethylaminophenyl)pyrazoline

(367) 1-[pyridyl-(3)]-3-(4-methoxystyryl)-5-(4-N,N-dibenzylaminophenyl)pyrazoline

(368) 1-[pyridyl-(3)]-3-(4-methoxystyryl)-5-(4-N,N-dipropylaminophenyl)pyrazoline

(369) 1-[pyridyl-(3)]-3-(4-methoxystyryl)-5-(4-N-ethyl-N-benzylaminostyryl)pyrazoline

(370) 1-[pyridyl-(3)]-3-(4-methoxystyryl)-5-(4-N,N-dibutylaminostyryl)pyrazoline

(371) 1-[pyridyl-(3)]-3-(4-methoxystyryl)-5-(4-methoxyphenyl)pyrazoline

(372) 1-[pyridyl-(3)]-3,5-di-(4-methoxyphenyl)pyrazoline

(373) 1-[pyridyl-(3)]-3-(4-phenoxyxstyryl)-5-(4-N,N-diethylaminophenyl)pyrazoline

(374) 1-[2-methylpyridyl-(3)]-3-(4-methoxystyryl)-5-(4-methoxyphenyl)pyrazoline

(375) 1-[2-ethylpyridyl-(3)]-3-(4-methoxystyryl)-5-(4-methoxyphenyl)pyrazoline

(376) 1-[pyridyl-(3)]-3-(4-ethoxystyryl)-5-(4-ethoxyphenyl)pyrazoline

(377) 1-[quinolyl-(2)]-3-(4-methoxystyryl)-5-(4-N,N-dimethylaminophenyl)pyrazoline

(378) 1-[quinolyl-(2)]-3-(4-methoxystyryl)-5-(4-N,N-diethylaminophenyl)pyrazoline

(379) 1-[quinolyl-(2)]-3-(4-methoxystyryl)-5-(4-N,N-dibenzylaminophenyl)pyrazoline

(380) 1-[quinolyl-(2)]-3-(4-methoxystyryl)-5-(4-N,N-dipropylaminophenyl)pyrazoline

(381) 1-[quinolyl-(2)]-3-(4-methoxystyryl)-5-(4-N-ethyl-N-benzylaminostyryl)pyrazoline

(382) 1-[quinolyl-(2)]-3-(4-methoxystyryl)-5-(4-N,N-dibutylaminostyryl)pyrazoline

(383) 1-[quinolyl-(2)]-3-(4-methoxystyryl)-5-(4-methoxyphenyl)pyrazoline

(384) 1-[quinolyl-(2)]-3,5-di-(4-methoxyphenyl)-pyrazoline

(385) 1-[quinolyl-(2)]-3-(4-phenoxyxstyryl)-5-(4-N,N-diethylaminophenyl)pyrazoline

(386) 1-[quinolyl-(2)]-3-(4-ethoxystyryl)-5-(4-ethoxyphenyl)pyrazoline

(387) 1-[quinolyl-(2)]-3-(4-methoxystyryl)-5-(4-methoxyphenyl)pyrazoline

(388) 1-[quinolyl-(2)]-3-(4-methoxystyryl)-

-continued

- 5-4-(ethoxyphenyl)pyrazoline  
 (389) 1-[epidyl-(2)]-3-(4-methoxystyryl)-  
 5-(4-N,N-dimethylaminophenyl)pyrazoline  
 5 (390) 1-[epidyl-(2)]-3-(4-methoxystyryl)-  
 5-(4-N,N-diethylaminophenyl)pyrazoline  
 (391) 1-[epidyl-(2)]-3-(4-methoxystyryl)-  
 5-(4-N,N-dibenzylaminophenyl)pyrazoline  
 (392) 1-[epidyl-(2)]-3-(4-methoxystyryl)-  
 5-(4-N,N-dipropylaminophenyl)pyrazoline  
 10 (393) 1-[epidyl-(2)]-3-(4-methoxystyryl)-  
 5-(4-N-ethyl-N-benzylaminostyryl)pyrazoline  
 (394) 1-[epidyl-(2)]-3-(4-methoxystyryl)-  
 5-(4-N,N-dibutylaminostyryl)pyrazoline  
 (395) 1-[epidyl-(2)]-3-(4-methoxystyryl)-  
 5-(4-methoxyphenyl)pyrazoline  
 15 (396) 1-[epidyl-(2)]-3,5-di-(4-methoxy-  
 phenyl)pyrazoline  
 (397) 1-[epidyl-(2)]-3-(4-phenoxyxystyryl)-  
 5-(4-N,N-diethylaminophenyl)pyrazoline  
 (398) 1-[epidyl-(2)]-3-(4-ethoxystyryl)-  
 5-(4-ethoxyphenyl)pyrazoline  
 20 (399) 1-[epidyl-(2)]-3-(4-methoxystyryl)-  
 5-(4-methoxyphenyl)pyrazoline  
 (400) 1-[epidyl-(2)]-3-(4-methoxystyryl)-  
 5-(4-ethoxyphenyl)pyrazoline  
 (401) 1-[6-methoxypyridyl-(2)]-3-(4-methoxy-  
 styryl)-5-(4-N,N-dimethylaminophenyl)pyrazoline  
 25 (402) 1-[pyridyl-(2)]-3-(4-methoxystyryl)-  
 5-(4-N,N-diethylaminophenyl)pyrazoline  
 (403) 1-[pyridyl-(2)]-3-(4-methoxystyryl)-  
 5-(4-N,N-dibenzylaminophenyl)pyrazoline  
 (404) 1-[pyridyl-(2)]-3-(4-methoxystyryl)-  
 5-(4-N,N-dipropylaminophenyl)pyrazoline  
 (405) 1-[pyridyl-(2)]-3-(4-methoxystyryl)-  
 5-(4-N-ethyl-N-benzylaminostyryl)pyrazoline  
 30 (406) 1-[pyridyl-(2)]-3-(4-methoxystyryl)-  
 5-(4-N,N-dibutylaminostyryl)pyrazoline  
 (407) 1-[pyridyl-(2)]-3-(4-methoxystyryl)-  
 5-(4-methoxyphenyl)pyrazoline  
 (408) 1-[pyridyl-(2)]-3,5-di-(4-methoxyphenyl)-  
 pyrazoline  
 35 (409) 1-[pyridyl-(2)]-3-(4-phenoxyxystyryl)-  
 5-(4-N,N-diethylaminophenyl)pyrazoline  
 (410) 1-[pyridyl-(2)]-3-(4-ethoxystyryl)-  
 5-(4-ethoxyphenyl)pyrazoline  
 (411) 1-[pyridyl-(2)]-3-(4-methoxystyryl)-5-  
 (4-methoxyphenyl)pyrazoline  
 40 (412) 1-[pyridyl-(2)]-3-(4-methoxystyryl)-5-  
 (4-ethoxyphenyl)pyrazoline  
 (413) 1-[N-ethyl-carbazolyl-(3)]-3-(4-methoxy-  
 styryl)-5-(4-N,N-diethylaminophenyl)pyrazoline  
 (414) 1-[N-ethyl-carbazolyl-(3)]-3-(4-methoxy-  
 styryl)-5-(4-methoxyphenyl)pyrazoline

45 These compounds are also readily prepared by known synthetic methods, for instance, by refluxing an unsaturated ketone and a hydrazino compound represented by the following formulae (i) and (j), respectively, in alcohol in the presence of a small amount of 50 acetic acid for several hours.

## Formula

- 55 (i)  $R_2-CH=CH-C(=O)-C=C=CH)_n-R_1$   
 (ii)  $X_1-NH-NH_2$   
 (R<sub>1</sub>, R<sub>2</sub>, X<sub>1</sub>, and n are as defined above)

$$\textcircled{1} \quad \text{X}_1-\text{NH}-\text{NH}_2$$

60 (R<sub>1</sub>, R<sub>2</sub>, X<sub>1</sub>, and n are as defined above)

- (415) 1-[pyridyl-(3)-3,5-di-(4-N,N-dimethyl-  
aminostyryl)pyrazoline  
65 (416) 1-[pyridyl-(3)-3,5-di-(4-N,N-diethyl-  
aminostyryl)pyrazoline  
(417) 1-[pyridyl-(3)-3,5-di-(4-N,N-dibenzyl-  
aminostyryl)pyrazoline  
(418) 1-[pyridyl-(3)-3,5-di-(4-N,N-dipropyl-

-continued

- (419) aminostyryl)pyrazoline  
 1-[pyridyl-(3)]-3,5-di-(4-N,N—dibutyl)-  
 aminostyryl)pyrazoline
- (420) 1-[pyridyl-(3)]-3-(4-N,N—diethylamino-  
 styryl)-5-(4-N,N—dibenzylaminostyryl)pyrazoline
- (421) 1-[pyridyl-(3)]-3-( $\alpha$ -methyl-4-N,N—  
 diethylaminostyryl)-5-(4-N,N—diethylaminostyryl)-  
 pyrazoline
- (422) 1-[pyridyl-(3)]-3-( $\alpha$ -benzyl-4-N,N—  
 diethylaminostyryl)-5-(4-N,N—diethylaminostyryl)-  
 pyrazoline
- (423) 1-[pyridyl-(3)]-3-( $\alpha$ -phenyl-4-N,N—  
 diethylaminostyryl)-5-(4-N,N—diethylaminostyryl)-  
 pyrazoline
- (424) 1-[pyridyl-(3)]-3,5-di-(4-N,N—  
 diethylaminostyryl)-4-methylpyrazoline
- (425) 1-[pyridyl-(3)]-3,5-di-(4-N,N—  
 diethylaminostyryl)-4-benzylpyrazoline
- (426) 1-[pyridyl-(3)]-3,5-di-(4-N,N—  
 diethylaminostyryl)-4-phenylpyrazoline
- (427) 1-[pyridyl-(3)]-3-(4-N,N—diethylamino-  
 phenyl)-4-methyl-5-(4-N,N—diethylaminostyryl)pyrazoline
- (428) 1-[pyridyl-(3)]-3-[ $\beta$ -(2-furyl)vinyl]-  
 5-(4-N,N—diethylaminostyryl)pyrazoline
- (429) 1-[pyridyl-(3)]-3-[ $\beta$ -(N—ethyl-4-  
 imidazolyl)vinyl]-5-(4-N,N—diethylaminostyryl)-  
 pyrazoline
- (430) 1-[pyridyl-(3)]-3-[ $\beta$ -(N—ethyl-3-  
 carbazolyl)vinyl]-5-(4-N,N—diethylaminostyryl)-  
 pyrazoline
- (431) 1-[pyridyl-(3)]-3-(4-N,N—diethyl-  
 aminostyryl)-5-[ $\beta$ -(2-furyl)vinyl]pyrazoline
- (432) 1-[pyridyl-(3)]-3-(4-N,N—diethyl-  
 aminostyryl)-5-[ $\beta$ -(N—ethyl-4-imidazolyl)vinyl]-  
 pyrazoline
- (433) 1-[pyridyl-(3)]-3-(4-N,N—diethyl-  
 aminostyryl)-5-[ $\beta$ -(N—ethyl-4-oxazolyl)vinyl] -  
 pyrazoline
- (434) 1-[pyridyl-(3)]-3,5-di-[ $\beta$ -(2-furyl)-  
 vinyl]pyrazoline
- (435) 1-[pyridyl-(3)]-3,5-di-(4-methoxystyryl)-  
 pyrazoline
- (436) 1-[quinolyl-(2)]-3,5-di-(4-N,N—  
 dimethylaminostyryl)pyrazoline
- (437) 1-[quinolyl-(2)]-3,5-di-(4-N,N—  
 diethylaminostyryl)pyrazoline
- (438) 1-[quinolyl-(2)]-3,5-di-(4-N,N—  
 dibenzylaminostyryl)pyrazoline
- (439) 1-[quinolyl-(2)]-3,5-di-(4-N,N—  
 dipropylaminostyryl)pyrazoline
- (440) 1-[quinolyl-(2)]-3,5-di-(4-N,N—  
 dibutylaminostyryl)pyrazoline
- (441) 1-[quinolyl-(2)]-3-(4-N,N—diethylamino-  
 styryl)-5-(4-N,N—dibenzylaminostyryl)pyrazoline
- (442) 1-[quinolyl-(2)]-3-( $\alpha$ -methyl-4-N,N—  
 diethylaminostyryl)-5-(4-N,N—diethylaminostyryl)-  
 pyrazoline
- (443) 1-[quinolyl-(2)]-3-( $\alpha$ -benzyl-4-N,N—  
 diethylaminostyryl)-5-(4-N,N—diethylaminostyryl)-  
 pyrazoline
- (444) 1-[quinolyl-(2)]-3-( $\alpha$ -phenyl-4-N,N—  
 diethylaminostyryl)-5-(4-N,N—diethylaminostyryl)-  
 pyrazoline
- (445) 1-[quinolyl-(2)]-3,5-di-(4-N,N—  
 diethylaminostyryl)-4-methylpyrazoline
- (446) 1-[quinolyl-(2)]-3,5-di-(4-N,N—  
 diethylaminostyryl)-4-benzylpyrazoline
- (447) 1-[quinolyl-(2)]-3,5-di-(4-N,N—  
 diethylaminostyryl)-4-phenylpyrazoline
- (448) 1-[quinolyl-(2)]-3-(4-N,N—diethylamino-  
 phenyl)-4-methyl-5-(4-N,N—diethylaminostyryl)pyrazoline
- (449) 1-[quinolyl-(2)]-3-[ $\beta$ -(2-furyl)vinyl]-  
 5-(4-N,N—diethylaminostyryl)pyrazoline
- (450) 1-[quinolyl-(2)]-3-[ $\beta$ -(N—ethyl-4-  
 imidazolyl)vinyl]-5-(4-N,N—diethylaminostyryl)-  
 pyrazoline
- (451) 1-[quinolyl-(2)]-3-[ $\beta$ -(N—ethyl-3-  
 carbazolyl)vinyl]-5-(4-N,N—diethylaminostyryl)-  
 pyrazoline
- (452) 1-[quinolyl-(2)]-3-(4-N,N—diethylamino-  
 styryl)-5-[ $\beta$ -(2-furyl)vinyl]pyrazoline
- (453) 1-[quinolyl-(2)]-3-(4-N,N—diethylamino-

-continued

- styryl)-5-[ $\beta$ -(N—ethyl-4-imidazolyl)vinyl]pyrazoline
- (454) 1-[quinolyl-(2)]-3-(4-N,N—diethylamino-  
 styryl)-5-[ $\beta$ -(N—ethyl-4-oxazolyl)vinyl]pyrazoline
- 5 (455) 1-[quinolyl-(2)]-3,5-di-[ $\beta$ -(2-furyl)-  
 vinyl]pyrazoline
- (456) 1-[quinolyl-(2)]-3,5-di-(4-methoxy-  
 styryl)pyrazoline
- (457) 1-[lepidyl-(2)]-3,5-di-(4-N,N—  
 dimethylaminostyryl)pyrazoline
- 10 (458) 1-[lepidyl-(2)]-3,5-di-(4-N,N—  
 diethylaminostyryl)pyrazoline
- (459) 1-[lepidyl-(2)]-3,5-di-(4-N,N—  
 dibenzylaminostyryl)pyrazoline
- (460) 1-[lepidyl-(2)]-3,5-di-(4-N,N—  
 dipropylaminostyryl)pyrazoline
- 15 (461) 1-[lepidyl-(2)]-3,5-di-(4-N,N—  
 dibutylaminostyryl)pyrazoline
- (462) 1-[lepidyl-(2)]-3-(4-N,N—diethylamino-  
 styryl)-5-(4-N,N—dibenzylaminostyryl)pyrazoline
- (463) 1-[lepidyl-(2)]-3-( $\alpha$ -methyl-4-N,N—  
 diethylaminostyryl)-5-(4-N,N—diethylaminostyryl)-  
 pyrazoline
- 20 (464) 1-[lepidyl-(2)]-3-( $\alpha$ -benzyl-4-N,N—  
 diethylaminostyryl)-5-(4-N,N—diethylaminostyryl)-  
 pyrazoline
- (465) 1-[lepidyl-(2)]-3-( $\alpha$ -phenyl-4-N,N—  
 diethylaminostyryl)-5-(4-N,N—diethylaminostyryl)-  
 pyrazoline
- 25 (466) 1-[lepidyl-(2)]-3,5-di-(4-N,N—  
 diethylaminostyryl)-4-methylpyrazoline
- (467) 1-[lepidyl-(2)]-3,5-di-(4-N,N—  
 diethylaminostyryl)-4-benzylpyrazoline
- (468) 1-[lepidyl-(2)]-3,5-di-(4-N,N—  
 diethylaminostyryl)-4-phenylpyrazoline
- 30 (469) 1-[lepidyl-(2)]-3-(4-N,N—diethylamino-  
 phenyl)-4-methyl-5-(4-N,N—diethylaminostyryl)pyrazoline
- (470) 1-[lepidyl-(2)]-3-[ $\beta$ -(2-furyl)vinyl]-  
 5-(4-N,N—diethylaminostyryl)pyrazoline
- (471) 1-[lepidyl-(2)]-3-[ $\beta$ -(N—ethyl-4-  
 imidazolyl)vinyl]-5-(4-N,N—diethylaminostyryl)-  
 pyrazoline
- 35 (472) 1-[lepidyl-(2)]-3-[ $\beta$ -(N—ethyl-3-  
 carbazolyl)vinyl]-5-(4-N,N—diethylaminostyryl)-  
 pyrazoline
- (473) 1-[lepidyl-(2)]-3-(4-N,N—diethylamino-  
 styryl)-5-[ $\beta$ -(2-furyl)vinyl]pyrazoline
- 40 (474) 1-[lepidyl-(2)]-3-(4-N,N—diethylamino-  
 styryl)-5-[ $\beta$ -(N—ethyl-4-imidazolyl)vinyl]pyrazoline
- (475) 1-[lepidyl-(2)]-3-(4-N,N—diethylamino-  
 styryl)-5-[ $\beta$ -(N—ethyl-4-oxazolyl)vinyl]pyrazoline
- (476) 1-[lepidyl-(2)]-3,5-di-[ $\beta$ -(2-furyl)vinyl]-  
 pyrazoline
- 45 (477) 1-[lepidyl-(2)]-3,5-di-(4-methoxystyryl)-  
 pyrazoline
- (478) 1-[pyridyl-(2)]-3,5-di-(4-N,N—  
 dimethylaminostyryl)pyrazoline
- (479) 1-[pyridyl-(2)]-3,5-di-(4-N,N—  
 diethylaminostyryl)pyrazoline
- 50 (480) 1-[pyridyl-(2)]-3,5-di-(4-N,N—  
 dibenzylaminostyryl)pyrazoline
- (481) 1-[pyridyl-(2)]-3,5-di-(4-N,N—  
 dipropylaminostyryl)pyrazoline
- (482) 1-[pyridyl-(2)]-3,5-di-(4-N,N—  
 dibutylaminostyryl)pyrazoline
- 55 (483) 1-[pyridyl-(2)]-3-(4-N,N—diethylamino-  
 styryl)-5-(4-N,N—dibenzylaminostyryl)pyrazoline
- (484) 1-[pyridyl-(2)]-3-( $\alpha$ -methyl-4-N,N—  
 diethylaminostyryl)-5-(4-N,N—diethylaminostyryl)-  
 pyrazoline
- (485) 1-[pyridyl-(2)]-3-( $\alpha$ -benzyl-4-N,N—  
 diethylaminostyryl)-5-(4-N,N—diethylaminostyryl)-  
 pyrazoline
- 60 (486) 1-[pyridyl-(2)]-3-( $\alpha$ -phenyl-4-N,N—  
 diethylaminostyryl)-5-(4-N,N—diethylaminostyryl)-  
 pyrazoline
- (487) 1-[pyridyl-(2)]-3,5-di-(4-N,N—  
 diethylaminostyryl)-4-methylpyrazoline
- 65 (488) 1-[pyridyl-(2)]-3,5-di-(4-N,N—  
 diethylaminostyryl)-4-benzylpyrazoline
- (489) 1-[pyridyl-(2)]-3,5-di-(4-N,N—  
 diethylaminostyryl)-4-phenylpyrazoline
- (490) 1-[pyridyl-(2)]-3-(4-N,N—

-continued

- diethylaminophenyl)-4-methyl-5-(4-N,N—  
diethylaminostyryl)pyrazoline  
(491) 1-[pyridyl-(2)]-3-[ $\beta$ -(2-furyl)vinyl]-  
5-(4-N,N—diethylaminostyryl)pyrazoline  
(492) 1-[pyridyl-(2)]-3-[ $\beta$ -(N-ethyl-4-  
imidazolyl)vinyl]-5-(4-N,N—diethylaminostyryl)-  
pyrazoline  
(493) 1-[pyridyl-(2)]-3-[ $\beta$ -(N-ethyl-3-  
carbazolyl)vinyl]-5-(4-N,N—diethylaminostyryl)-  
pyrazoline  
(494) 1-[pyridyl-(2)]-3-(4-N,N—diethylamino-  
styryl)-5-[ $\beta$ -(2-furyl)vinyl]pyrazoline  
(495) 1-[pyridyl-(2)]-3-(4-N,N—diethylamino-  
styryl)-5-[ $\beta$ -(N-ethyl-4-imidazolyl)vinyl]pyrazoline  
(496) 1-[pyridyl-(2)]-3-(4-N,N—diethylamino-  
styryl)-5-[ $\beta$ -(N-ethyl-4-oxazolyl)vinyl]pyrazoline  
(497) 1-[pyridyl-(2)]-3,5-di-[ $\beta$ -(2-furyl)vinyl]-  
pyrazoline  
(498) 1-[pyridyl-(2)]-3,5-di-(4-methoxystyryl)-  
pyrazoline  
(499) 1-[N-ethyl-carbazolyl-(3)]-3,5-di-(4-  
N,N—diethylaminostyryl)pyrazoline  
(500) 1-[N-ethyl-carbazolyl-(3)]-3,5-di-  
(4-N,N—diethylaminostyryl)-4-methylpyrazoline  
(501) 1-[6-methoxypyridyl-(2)]-3,5-di-  
(4-morpholinostyryl)pyrazoline  
(502) 1-[6-methoxypyridyl-(2)]-3,5-di-  
(4-pyrrolidinostyryl)pyrazoline

5

10

15

25

These compounds are readily prepared by known  
synthetic methods, for instance, by refluxing an unsatu-  
rated ketone and a hydrazino compound represented by  
the following formulae (k) and (l), respectively, in alco-  
hol in the presence of a small amount of acetic acid for  
several hours.

Formula



30

35



40

(R<sub>1</sub>, R<sub>2</sub>, R<sub>4</sub>, R<sub>5</sub>, X<sub>1</sub>, and n are as defined above)



45



55

60

65



(505)



(506)



(507)



(508)



(509)

-continued



-continued

(510)

5



(511) 15

20



25

30

35

40

45

50

55

(512)

60

65



(513)

50

55

(514)

60

65



(515)

(516)

(517)

(518)

(519)

-continued



(520)

-continued



(521)

(522)

(523)

(524)

(525)

(526)

(527)

(528)

(529)

These compounds are readily prepared by ring closure of compounds represented by the following formulas (m) and (n) by, for example, the method disclosed in Japanese Patent Kokai No. 26761(1973).

Formula

(m)



(n)



(R<sub>1</sub>, R<sub>4</sub>, R<sub>11</sub>, R<sub>12</sub>, X<sub>1</sub>, I, Z, and n are as defined above, and Y is an acidic residue.)



27

-continued



28

-continued



(533) 30 These compounds are readily prepared by ring closure of compounds represented by the following formulae (o) and (p) by, for example, the method disclosed in Japanese Patent Kokai No. 26761(1973).

35

## Formula

(c)



$$\text{X}_1-\text{NH}-\text{N}=\text{C}(\text{Y})-\text{C}(\text{R}_4)=\text{CH}-\text{R}_1$$

(R<sub>1</sub>, R<sub>4</sub>, R<sub>11</sub>, R<sub>12</sub>, X<sub>1</sub>, Z<sub>1</sub> and I are as defined above, and Y is an acidic residue.)



(538)

-continued



(539)



(540)



(541)



(542)



(543)

-continued

(544)



(545)



(546)



(547)



(548)



-continued

(549)



(550)



(551)



(552)



-continued

(553)



(554)



(555)



(556)



(557)



-continued



(558)



(559)



(560)



(561)



(562)

-continued

(563)



(564)



(565)



(566)



(567)

These compounds are readily prepared by known 65 in the presence a small amount of acetic acid for several methods, for instance, by refluxing an unsaturated ketone and a hydrazino compound represented by the following formulae (q) and (r), respectively, in alcohol

Formula



wherein  $\text{R}_6$ ,  $\text{R}_7$ ,  $\text{R}_8$ ,  $\text{R}_9$ ,  $\text{R}_{10}$ , and  $\text{X}_2$  are as defined above, and  $\text{X}_2$  and  $\text{X}_3$  are the same.

The pyrazoline, spiropyrazoline, and bispyrazoline compounds cited above may be used singly or in combination.

In preferred embodiments of the electrophotographic photosensitive member of this invention, laminated photosensitive layers are used which comprises a charge transport layer containing the foregoing pyrazoline compound as a charge-transporting material and a charge generation layer, which will be explained later.

The charge transport layer is preferably formed by coating and drying a solution prepared by dissolving said pyrazoline compound and a binder in a suitable solvent. Binders herein used include, for example, acrylic resins, methacrylic resins, vinyl chloride resin, vinyl acetate resin, phenolic resins, epoxy resins, polyester resins, polysulfone, alkyd resins, polycarbonates, polyurethanes, and copolymer resins containing two or more types of repeating units of these resins, among which polyester resins and polycarbonates are particularly preferred. Photoconductive polymers like poly(*N*-vinylcarbazole) can also be used as the binder which have a charge-transporting function per se.

Suitable compounding ratios of the charge-transporting compound to the binder are 10-500:100 by weight. Thickness of the charge transport layer is 2 to 100 $\mu$ , preferably 5-30 $\mu$ .

Solvents for the coating solution used for forming the charge transport layer include a number of useful organic solvents conventionally used. Typical examples thereof are aromatic hydrocarbons and their halogen derivatives such as benzene, toluene, xylene, and chlorobenzene; ketones such as acetone and 2-butanone; halogenated aliphatic hydrocarbons such as methylene chloride, chloroform, and ethylene chloride; cyclic or

linear ethers such as tetrahydrofuran and ethyl ether; and mixtures of these solvents.

Various additives can be incorporated into the charge transport layer of this invention. Such additives include diphenyl, chlorodiphenyl, o-terphenyl, p-terphenyl, dibutyl phthalate, dimethyl glycol phthalate, dioctyl phthalate, triphenyl phosphate, methylnaphthalene, benzophenone, chlorinated paraffin, dilaury thiopropionate, 3,5-dinitrosalicylic acid, various kinds of fluorocarbons, silicone oils, etc.

For the charge-generation layer, any charge-generating material can be used so far as it, on absorbing light, generates charge carriers in a very high efficiency. Preferred charge-generating materials in this invention

15 are inorganic substances including selenium, selenium-tellurium, selenium-arsenic, cadmium sulfide, and amorphous silicon and organic substances including pyrilium dyes, thiopyrilium dyes, triaryl methane dyes, thiazine dyes, cyanine dyes, phthalocyanine pigments, perylene pigments, indigo pigments, thioindigo pigments, quinacridone pigments, squaric acid pigments, azo pigments, polycyclic quinone pigments, and the like. Thickness of the charge generation layer is up to 5 $\mu$ , preferably 0.05 to 3 $\mu$ .

20 25 The charge generation layer is formed in an appropriate way such as vacuum deposition, sputtering, glow discharge, usual coating, and the like, to meet the nature of charge-generating material used.

Charge-generating materials are applied to coating 30 without any binder or in the form of dispersion in a binder solution or in the form of homogeneous solution along with a binder. In the above cases, the binder content in the charge generation layer should be up to 80%, preferably up to 40%, since excessive contents of binder adversely affect the sensitivity.

Binders available for the charge generation layer include poly(vinyl butyral), poly(methyl methacrylate), polyesters, poly(vinylidene chloride), chlorinated rubbers, polyvinyltoluene, styrene-maleic anhydride copolymer, polystyrene, poly(vinyl chloride), methylcellulose, polyamides, polyvinylpyridine, styrene-butadiene copolymer, etc.

The following compounds can be used as the charge 40 45 generating material for the electrophotographic photosensitive member of this invention.

Charge generating materials

Amorphous silicon  
Selenium-Tellurium  
Selenium-Arsenic



-continued

Charge generating materials

-continued  
Charge generating materials



(10)



(11)



(12)



(13)



(14)



(15)

-continued

Charge generating materials

(16)



(17)



(18)



(19)



(20)

-continued

Charge generating materials

(21)



(22)



(23)



(24)



(25)



(26)



-continued  
Charge generating materials



(27)



(28)



(29)



(30)

Copper phthalocyanine  
Cadmium sulfide

(31)

(32)

The above-cited pigments can be used singly or in combination, and in any crystal form,  $\alpha$ ,  $\beta$ , or others, of which the  $\beta$ -form is preferable.

The electrophotographic photosensitive member of this invention can be prepared by overlaying a suitable substrate with a charge generation layer containing the above-cited pigment and laminating a charge transport layer on this charge generation layer. This type of electrophotographic photosensitive member may also be provided with an intermediate layer between the substrate and the charge generation layer. This intermediate layer, when the photosensitive layers of laminate structure is charged, bars the injection of free charges from the conductive substrate into the photosensitive layers and acts at the same time as a bond layer to hold the photosensitive layers and the conductive layer en masse. The intermediate layer can be formed from a metal oxide such as aluminum oxide or a polymer such as polyethylene, polypropylene, acrylic resins, methacrylic resins, vinyl chloride resin, phenolic resins, epoxy resins, polyester resins, alkyd resins, polycarbonates, polyurethanes, polyimide resins, vinylidene chloride resin, vinyl chloride-vinyl acetate copolymer, casein, gelatin, poly(vinyl alcohol), ethyleneacrylic acid copolymer, nitrocellulose, and the like. Thickness of the intermediate or bond layer is 0.1 to 5 $\mu$ , preferably 0.5 to 3 $\mu$ . A laminate structure wherein the charge generation layer is laid on the upper side of the charge transport

layer is also acceptable. In this case, a suitable protective top coat may be formed.

For dispersing the pigment, known means can be applied such as ball mills, attritors, and the like, where the pigment particle size is reduced to 5 $\mu$  or less, preferably 2 $\mu$  or less, and most preferably 0.5 $\mu$  or less.

The pigment can also be applied after dissolved in an amine type of solvent such as ethylene diamine, and the like. The coating is carried out by a usual method such as blade coating, Meyer bar coating, spray coating, dip coating, and the like.

The charge generation layer surface can be mirror-finished, if necessary, for uniforming the carrier injection from the charge generation layer to the upper charge transport layer.

The charge transport layer is formed on the charge generation layer thus prepared. When the charge-transporting material has no film forming property, it is dissolved together with a binder in a suitable organic solvent and this coating solution is applied and dried in a usual way to form the charge transport layer.

Another embodiment of the electrophotographic photosensitive member of this invention comprises a conductive layer and a photosensitive layer formed thereon from a dispersion of said charge-generating material in a charge-transporting medium which comprises said pyrazoline compound as a charge-transporting material and an insulating binder [alternatively, said

medium comprises a binder, such as poly(N-vinylcarbazole), which also functions as a charge-transporting material. Insulating binders usable in this case include, for example, those disclosed in Japanese Patent Kokai Nos. 30328/1972 and 18545/1972 (corresponding to U.S. Pat. Nos. 3,894,868 and 3,870,516, respectively).

Substrates for use in the electrophotographic photosensitive member of this invention may be of any type existing so far as it is provided with conductivity. They include, for example, metallic sheets of aluminum, vanadium, molybdenum, chromium, cadmium, titanium, nickel, copper, zinc, palladium, indium, tin, platinum, gold, stainless steel, and brass and plastic sheets on which a metal is vacuum-deposited or a metal foil is laminated.

The electrophotographic photosensitive member of this invention is available not only for electrophotographic copying machines but also over wide fields of electrophotographic application such as those of laser printers, CRT printers, and electrophotographic printing plate making systems.

The electrophotographic photosensitive member according to this invention has outstandingly high sensitivity as compared with those employing conventional organic photoconductive materials and additionally it does not cause an increase in light area potential or a decrease in dark area potential even when its charging and exposure are repeated 10,000 times or more.

This invention will be illustrated referring to the following Examples:

#### EXAMPLES 1-9

A solution of defatted casein in an aqueous ammonia (casein 11.2 g, 28% aqueous ammonia 1 g, water 222 ml) was coated by means of a Meyer bar on an aluminum sheet and dried to form a bond layer of 1.0 g/m<sup>2</sup>.

A dispersion of 5 g of a disazo pigment having the following structure in a solution of 2 g of a butyral resin (butyral conversion degree 63 mol%) in 95 ml of ethanol was prepared by mixing in a ball mill for 40 hours and was coated by means of a Meyer bar on said bond layer to form a charge generation layer of 0.2 g/m<sup>2</sup> after drying.

Disazo pigment (pigment No. 10 cited above)



A solution prepared by dissolving 5 g of a pyrazoline compound shown in Table 1 and 5 g of a polycarbonate of bisphenol A (mol.wt. about 30,000) in 70 ml of tetrahydrofuran was coated on said charge generation layer and dried to form a charge transport layer of 10 g/m<sup>2</sup>.

Electrophotographic photosensitive members containing different pyrazoline compounds, thus prepared were tested for charge bearing characteristics by the following methods. They were moisture-conditioned at 20° C. and 65% R.H., corona-charged at  $\pm 5$  KV in the static fashion using an electrostatic copying paper test-

ing machine (Model SP-428, mfd. by Kawaguchi Denki K.K.), and after 10-second standing at the dark, were exposed to light at an intensity of 5 lux.

Charge bearing characteristics of these photosensitive members thus examined are shown in Table 1, wherein  $V_o$  is initial potential (-volt) produced by the charging,  $V_K$  is percentage retention of the potential after standing for 10 seconds at the dark, and  $E_{\frac{1}{2}}$  is exposure quantity (lux.sec) for halving the initial potential.

TABLE 1

| Example No. | Pyrazoline | $V_o$ (volt) | $V_K$ (%) | $E_{\frac{1}{2}}$ (lux.sec) |
|-------------|------------|--------------|-----------|-----------------------------|
| 15 1        | No. (2)    | -620         | 92        | 3.8                         |
| 2           | No. (62)   | -680         | 92        | 3.2                         |
| 3           | No. (166)  | -650         | 91        | 4.6                         |
| 4           | No. (285)  | -620         | 93        | 5.6                         |
| 5           | No. (371)  | -640         | 92        | 4.8                         |
| 6           | No. (416)  | -620         | 92        | 4.1                         |
| 7           | No. (503)  | -620         | 90        | 6.8                         |
| 8           | No. (523)  | -600         | 90        | 8.6                         |
| 9           | No. (531)  | -670         | 93        | 3.0                         |

Photosensitive members of these Examples each were attached onto a cylindrical drum, which was then set in a copying machine, wherein the drum is surrounded by a negative-charging device, light-irradiation optical system, development device, and charging device for transfer copying, so that image forming operations proceed successively as the drum revolves, to give images on sheets of transfer paper.

The photosensitive members of these Examples gave clear images at a light area exposure quantity of 15 lux.sec, and the images were good even when 25,000 or more copies were produced therewith.

#### EXAMPLES 10-169

Electrophotographic photosensitive members were prepared and tested for charge bearing characteristics, in the same manner as in Example 1 except for using pyrazoline compounds shown in Table 2 as charge-transporting materials in place of pyrazoline compound No. 2. The results are shown in Table 2.

TABLE 2

| Example No. | Pyrazoline | $V_o$ (volt) | $V_K$ (%) | $E_{\frac{1}{2}}$ (lux.sec) |
|-------------|------------|--------------|-----------|-----------------------------|
| 10          | No. (35)   | -640         | 92        | 3.2                         |
| 11          | No. (3)    | -610         | 92        | 6.7                         |
| 12          | No. (6)    | -600         | 93        | 6.1                         |
| 13          | No. (7)    | -550         | 90        | 4.8                         |
| 14          | No. (8)    | -560         | 92        | 5.0                         |
| 15          | No. (9)    | -520         | 90        | 7.0                         |
| 16          | No. (15)   | -630         | 92        | 3.1                         |
| 17          | No. (21)   | -520         | 92        | 7.3                         |
| 18          | No. (23)   | -580         | 90        | 6.5                         |

TABLE 2-continued

| Example No. | Pyrazoline | $V_o$ (volt) | $V_K$ (%) | $E \frac{1}{2}$ (lux.sec) |    |
|-------------|------------|--------------|-----------|---------------------------|----|
| 19          | No. (24)   | -570         | 92        | 5.8                       | 5  |
| 20          | No. (25)   | -550         | 91        | 6.2                       |    |
| 21          | No. (27)   | -670         | 93        | 3.0                       |    |
| 22          | No. (31)   | -580         | 92        | 6.3                       |    |
| 23          | No. (39)   | -550         | 90        | 6.5                       |    |
| 24          | No. (42)   | -520         | 90        | 6.7                       |    |
| 25          | No. (48)   | -650         | 93        | 3.0                       | 10 |
| 26          | No. (49)   | -600         | 90        | 4.4                       |    |
| 27          | No. (52)   | -550         | 90        | 6.1                       |    |
| 28          | No. (55)   | -520         | 91        | 6.7                       |    |
| 29          | No. (63)   | -600         | 90        | 6.6                       |    |
| 30          | No. (66)   | -640         | 92        | 4.1                       |    |
| 31          | No. (67)   | -630         | 91        | 3.8                       | 15 |
| 32          | No. (68)   | -650         | 93        | 4.0                       |    |
| 33          | No. (69)   | -580         | 90        | 6.1                       |    |
| 34          | No. (73)   | -550         | 92        | 6.7                       |    |
| 35          | No. (77)   | -680         | 90        | 3.0                       |    |
| 36          | No. (78)   | -620         | 92        | 4.7                       |    |
| 37          | No. (81)   | -640         | 90        | 3.2                       | 20 |
| 38          | No. (92)   | -630         | 92        | 3.0                       |    |
| 39          | No. (96)   | -650         | 92        | 4.0                       |    |
| 40          | No. (97)   | -610         | 90        | 5.2                       |    |
| 41          | No. (98)   | -600         | 92        | 6.3                       |    |
| 42          | No. (107)  | -670         | 92        | 3.0                       |    |
| 43          | No. (113)  | -680         | 92        | 3.0                       | 25 |
| 44          | No. (114)  | -610         | 93        | 6.4                       |    |
| 45          | No. (117)  | -660         | 92        | 4.2                       |    |
| 46          | No. (124)  | -670         | 90        | 3.8                       |    |
| 47          | No. (125)  | -600         | 92        | 6.2                       |    |
| 48          | No. (128)  | -640         | 90        | 4.2                       |    |
| 49          | No. (135)  | -650         | 92        | 3.7                       |    |
| 50          | No. (139)  | -620         | 90        | 4.9                       | 30 |
| 51          | No. (146)  | -670         | 92        | 3.1                       |    |
| 52          | No. (150)  | -620         | 90        | 4.7                       |    |
| 53          | No. (151)  | -610         | 92        | 6.6                       |    |
| 54          | No. (152)  | -600         | 90        | 6.5                       |    |
| 55          | No. (167)  | -600         | 90        | 5.2                       |    |
| 56          | No. (172)  | -620         | 91        | 5.0                       | 35 |
| 57          | No. (173)  | -610         | 92        | 4.8                       |    |
| 58          | No. (174)  | -610         | 90        | 4.6                       |    |
| 59          | No. (175)  | -600         | 92        | 5.2                       |    |
| 60          | No. (178)  | -580         | 90        | 6.2                       |    |
| 61          | No. (180)  | -590         | 91        | 4.7                       |    |
| 62          | No. (191)  | -650         | 92        | 3.2                       | 40 |
| 63          | No. (195)  | -660         | 91        | 3.3                       |    |
| 64          | No. (196)  | -600         | 90        | 4.9                       |    |
| 65          | No. (208)  | -580         | 91        | 5.7                       |    |
| 66          | No. (217)  | -610         | 92        | 5.2                       |    |
| 67          | No. (224)  | -640         | 92        | 3.4                       |    |
| 68          | No. (231)  | -590         | 90        | 6.6                       |    |
| 69          | No. (232)  | -580         | 90        | 5.2                       | 45 |
| 70          | No. (235)  | -570         | 90        | 6.0                       |    |
| 71          | No. (236)  | -580         | 92        | 6.1                       |    |
| 72          | No. (237)  | -560         | 90        | 6.8                       |    |
| 73          | No. (238)  | -570         | 90        | 7.1                       |    |
| 74          | No. (239)  | -570         | 91        | 6.8                       |    |
| 75          | No. (254)  | -650         | 90        | 3.1                       | 50 |
| 76          | No. (255)  | -600         | 90        | 4.6                       |    |
| 77          | No. (266)  | -580         | 92        | 5.9                       |    |
| 78          | No. (271)  | -570         | 90        | 6.3                       |    |
| 79          | No. (273)  | -600         | 91        | 4.7                       |    |
| 80          | No. (286)  | -610         | 92        | 5.2                       |    |
| 81          | No. (274)  | -580         | 90        | 7.6                       | 55 |
| 82          | No. (289)  | -610         | 92        | 4.1                       |    |
| 83          | No. (290)  | -620         | 90        | 4.0                       |    |
| 84          | No. (292)  | -620         | 92        | 3.6                       |    |
| 85          | No. (295)  | -570         | 90        | 8.2                       |    |
| 86          | No. (297)  | -600         | 92        | 6.1                       |    |
| 87          | No. (301)  | -560         | 90        | 8.3                       |    |
| 88          | No. (305)  | -650         | 90        | 3.1                       | 60 |
| 89          | No. (310)  | -630         | 92        | 4.5                       |    |
| 90          | No. (312)  | -620         | 90        | 6.3                       |    |
| 91          | No. (317)  | -620         | 93        | 5.4                       |    |
| 92          | No. (325)  | -640         | 90        | 4.7                       |    |
| 93          | No. (337)  | -600         | 90        | 6.6                       |    |
| 94          | No. (344)  | -620         | 92        | 7.3                       |    |
| 95          | No. (345)  | -650         | 90        | 3.7                       |    |
| 96          | No. (349)  | -600         | 90        | 7.0                       |    |
| 97          | No. (352)  | -580         | 92        | 7.6                       |    |
| 98          | No. (358)  | -570         | 90        | 8.2                       |    |

TABLE 2-continued

| Example No. | Pyrazoline | $V_o$ (volt) | $V_K$ (%) | $E \frac{1}{2}$ (lux.sec) |
|-------------|------------|--------------|-----------|---------------------------|
| 99          | No. (363)  | -550         | 92        | 8.7                       |
| 100         | No. (366)  | -630         | 93        | 4.2                       |
| 101         | No. (367)  | -650         | 91        | 5.1                       |
| 102         | No. (372)  | -620         | 92        | 5.8                       |
| 103         | No. (373)  | -580         | 90        | 7.6                       |
| 104         | No. (374)  | -630         | 91        | 3.6                       |
| 105         | No. (378)  | -650         | 90        | 4.1                       |
| 106         | No. (383)  | -630         | 90        | 7.8                       |
| 107         | No. (386)  | -600         | 92        | 6.9                       |
| 108         | No. (395)  | -620         | 90        | 6.0                       |
| 109         | No. (400)  | -640         | 92        | 4.3                       |
| 110         | No. (402)  | -600         | 90        | 5.6                       |
| 111         | No. (407)  | -620         | 92        | 3.2                       |
| 112         | No. (411)  | -630         | 93        | 4.0                       |
| 113         | No. (417)  | -580         | 90        | 7.9                       |
| 114         | No. (422)  | -600         | 92        | 6.5                       |
| 115         | No. (424)  | -610         | 91        | 4.2                       |
| 116         | No. (425)  | -590         | 93        | 5.6                       |
| 117         | No. (427)  | -610         | 90        | 5.8                       |
| 118         | No. (428)  | -550         | 90        | 8.0                       |
| 119         | No. (437)  | -610         | 92        | 4.0                       |
| 120         | No. (442)  | -600         | 90        | 5.9                       |
| 121         | No. (448)  | -570         | 90        | 7.8                       |
| 122         | No. (449)  | -560         | 91        | 8.2                       |
| 123         | No. (458)  | -620         | 93        | 3.8                       |
| 124         | No. (459)  | -570         | 90        | 7.6                       |
| 125         | No. (464)  | -580         | 91        | 8.3                       |
| 126         | No. (471)  | -570         | 92        | 7.9                       |
| 127         | No. (477)  | -550         | 90        | 8.4                       |
| 128         | No. (479)  | -640         | 90        | 4.1                       |
| 129         | No. (484)  | -600         | 92        | 4.9                       |
| 130         | No. (487)  | -570         | 90        | 7.7                       |
| 131         | No. (490)  | -560         | 91        | 8.3                       |
| 132         | No. (491)  | -550         | 90        | 8.5                       |
| 133         | No. (492)  | -560         | 90        | 7.8                       |
| 134         | No. (497)  | -550         | 90        | 8.6                       |
| 135         | No. (501)  | -620         | 92        | 4.3                       |
| 136         | No. (504)  | -600         | 92        | 8.2                       |
| 137         | No. (505)  | -630         | 90        | 5.5                       |
| 138         | No. (506)  | -660         | 92        | 3.2                       |
| 139         | No. (507)  | -650         | 91        | 4.6                       |
| 140         | No. (508)  | -620         | 92        | 6.6                       |
| 141         | No. (509)  | -660         | 92        | 3.2                       |
| 142         | No. (511)  | -650         | 90        | 5.2                       |
| 143         | No. (512)  | -600         | 90        | 8.9                       |
| 144         | No. (514)  | -620         | 91        | 7.8                       |
| 145         | No. (516)  | -650         | 90        | 6.8                       |
| 146         | No. (519)  | -600         | 90        | 10.2                      |
| 147         | No. (524)  | -610         | 90        | 9.3                       |
| 148         | No. (525)  | -630         | 90        | 6.4                       |
| 149         | No. (526)  | -620         | 91        | 5.1                       |
| 150         | No. (527)  | -640         | 90        | 5.5                       |
| 151         | No. (528)  | -590         | 89        | 8.8                       |
| 152         | No. (529)  | -620         | 91        | 4.7                       |
| 153         | No. (530)  | -600         | 90        | 7.8                       |
| 154         | No. (533)  | -600         | 92        | 7.6                       |
| 155         | No. (534)  | -610         | 90        | 8.7                       |
| 156         | No. (535)  | -620         | 93        | 7.9                       |
| 157         | No. (536)  | -620         | 91        | 12.6                      |
| 158         | No. (539)  | -600         | 90        | 6.7                       |
| 159         | No. (541)  | -630         | 92        | 5.1                       |
| 160         | No. (543)  | -650         | 92        | 3.8                       |
| 161         | No. (546)  | -580         | 91        | 7.8                       |
| 162         | No. (547)  | -570         | 90        | 8.3                       |
| 163         | No. (549)  | -690         | 92        | 3.2                       |
| 164         | No. (550)  | -590         | 91        | 8.0                       |
| 165         | No. (557)  | -630         | 92        | 4.2                       |
| 166         | No. (558)  | -670         | 93        | 3.3                       |
| 167         | No. (561)  | -680         | 93        | 3.0                       |
| 168         | No. (563)  | -600         | 92        | 8.8                       |
| 169         | No. (567)  | -640         | 91        | 4.7                       |

The photosensitive members of these Examples were also set in the copying machine used in Example 1 and images were formed therewith, with the result that clear images showing no fogging were obtained, and in addition the images were good even when 25,000 or more copies were produced therewith.

**EXAMPLES 170–178**

A charge generation layer  $0.15\mu$  thick was formed on an aluminum plate  $100\mu$  thick by vacuum deposition of perylene pigment of the following structure.

Electrophotographic photosensitive members were prepared and tested, in the same manner as in Examples 5 1-9 except for using a disazo pigment of the following structure as a charge-generating material in place of the disazo pigments used in Examples 1-9.

**EXAMPLES 179-187**



30



A solution prepared by dissolving 5 g of a polyester resin (Vylon 200, mfd. by Toyo Spinning Co., Ltd.) and 5 g of a pyrazoline compound shown in Table 3 in 150 ml of dichloromethane was coated on said charge generation layer and dried to form a charge transport layer of 11 g/m<sup>2</sup>.

Electrophotographic photosensitive members containing different pyrazoline compounds, thus prepared were tested for charge bearing characteristics in the same fashion as in Example 1. The results are shown in Table 3.

TABLE 3

| Example No. | Pyrazoline | $V_o$ (volt) | $V_K$ (%) | $E \frac{1}{2}$ (lux.sec) |
|-------------|------------|--------------|-----------|---------------------------|
| 170         | No. (2)    | -630         | 93        | 10.6                      |
| 171         | No. (62)   | -660         | 93        | 4.2                       |
| 172         | No. (166)  | -640         | 93        | 4.7                       |
| 173         | No. (285)  | -610         | 93        | 4.7                       |
| 174         | No. (371)  | -580         | 93        | 8.6                       |
| 175         | No. (416)  | -600         | 93        | 7.9                       |
| 176         | No. (503)  | -580         | 92        | 10.9                      |
| 177         | No. (523)  | -560         | 92        | 12.2                      |
| 178         | No. (531)  | -620         | 93        | 7.9                       |

These photosensitive members were also tested for durability in the same manner as in Example 1, giving good images up to 25,000 or more copies.

Charge bearing characteristics of these photosensitive members, measured in the same fashion as used in Examples 1-9 are shown in Table 4.

TABLE 4

| Example No. | Pyrazoline | V <sub>O</sub> (volt) | V <sub>K</sub> (%) | E $\frac{1}{2}$ (lux.sec) |
|-------------|------------|-----------------------|--------------------|---------------------------|
| 40          | 179        | No. (2)               | -640               | 93                        |
|             | 180        | No. (62)              | -680               | 93                        |
|             | 181        | No. (166)             | -570               | 90                        |
|             | 182        | No. (285)             | -600               | 93                        |
|             | 183        | No. (371)             | -600               | 90                        |
|             | 184        | No. (416)             | -600               | 90                        |
| 45          | 185        | No. (503)             | -680               | 93                        |
|             | 186        | No. (523)             | -600               | 92                        |
|             | 187        | No. (531)             | -660               | 90                        |

These photosensitive members were also tested for durability in the same manner as in Example 1, giving 50 good images up to 25,000 or more copies.

### EXAMPLES 188-196

55 A mixture of 20 g of a poly(N-vinylcarbazole), (mol. wt. about 300,000), 3.0 g of a pyrazoline compound shown in Table 5, 10 g of a polyester resin solution (solid content 20%, registered trade mark: Polyester Adhesive 490,000, mfd. by DuPont de Nemours & Co.), 2.0 g of a pigment of the following structure, and 60 180 ml of tetrahydrofuran were dispersed in a ball mill for 40 hours. The resulting dispersion was coated by means of an applicator on an aluminum coating vacuum-deposited on a Mylar film and dried to give a coating weight of 12 g/m<sup>2</sup>.

65 Electrophotographic photosensitive members prepared in this way were tested for charge bearing characteristics in the same fashion as described in Example 1 but the charging polarity was positive. The results are shown in Table 5.



TABLE 5

| Example No. | Pyrazoline | $V_o$ (volt) | $V_K$ (%) | $E \frac{1}{2}$ (lux.sec) |
|-------------|------------|--------------|-----------|---------------------------|
| 188         | No. (27)   | +440         | 82        | 12.9                      |
| 189         | No. (113)  | +470         | 84        | 13.8                      |
| 190         | No. (275)  | +490         | 86        | 14.2                      |
| 191         | No. (345)  | +460         | 89        | 12.6                      |
| 192         | No. (407)  | +450         | 84        | 18.6                      |
| 193         | No. (501)  | +450         | 83        | 16.6                      |
| 194         | No. (503)  | +470         | 88        | 14.6                      |
| 195         | No. (523)  | +480         | 90        | 15.2                      |
| 196         | No. (544)  | +460         | 86        | 15.7                      |

15

20

25

## EXAMPLES 197-205

A surface-cleaned molybdenum plate (substrate) 0.2 mm thick was fixed on a predetermined position of a glow discharge vacuum-deposition chamber. After the 30 chamber was evacuated to about  $5 \times 10^{-6}$  torr, the input voltage of a heater was raised and the molybdenum substrate temperature was settled to 150° C. Hydrogen gas and silane gas (15 vol.-% based on hydrogen gas) were introduced into the chamber and the chamber 35 pressure was settled to 0.5 torr by regulating the gas flow rates and a main valve of the chamber.

Then, 5 MHz high frequency power was applied to an induction coil to generate a glow discharge in an internal space, surrounded by the coil, of the chamber, 40 where the input power was 30 W. Under these conditions, amorphous silicon film was grown to a thickness of  $2\mu$ , and thereafter the glow discharge was stopped. The heater and the high frequency power source were turned off, and after the substrate temperature dropped 45 to 100° C., the hydrogen inlet valve and the silane inlet valve were turned off to evacuate the chamber to  $10^{-5}$  torr or less, then the chamber pressure was returned to the atmospheric value, and the substrate was taken out.

The same charge transport layer as each of Examples 50 1-9 was formed in the same manner as in Example 1 on each of amorphous silicon layers prepared by the above-mentioned procedure.

Photosensitive members thus obtained were set each in a charging and exposing testing machine, corona-charged at  $\pm 6$  KV, and immediately thereafter was 55 irradiated with a pattern of light which was projected by using a tungsten lamp through a transmission type of test chart.

Immediately thereafter, the members were cascaded 60 by a positive-working developer (containing toner and carrier) to obtain good images on the surfaces of the photosensitive members.

What we claim is:

1. An electrophotographic photosensitive member 65 comprising a charge generation layer and a charge transport layer which includes at least one pyrazoline compound represented by the following formula:



wherein  $X_1$  is a substituted or unsubstituted heterocyclic residue selected from the group consisting of substituted or unsubstituted pyridyl, quinolyl, carbazolyl, furyl, imidazolyl, oxazolyl, and isoxazolyl;  $R_1$  is a substituted or unsubstituted aryl or heterocyclic residue;  $R_4$  is hydrogen, a halogen, or a substituted or unsubstituted alkyl or aryl;  $R_{11}$  is a substituted or unsubstituted alkyl;  $R_{12}$  is hydrogen, a halogen, or an organic monovalent residue;  $Z$  is



or  $-\text{CH}=\text{CH}-$ , wherein  $R_{13}$  and  $R_{14}$  are each a substituted or unsubstituted alkyl;

$n$  is 0 or 1; and

1 is an integer of 1 to 4.

2. An electrophotographic photosensitive member of claim 1, wherein said  $R_1$  is a di-substituted aminophenyl.

3. An electrophotographic photosensitive member of claim 2, wherein said di-substituted aminophenyl is a dialkylaminophenyl.

4. An electrophotographic photosensitive member of claim 3, wherein said dialkylaminophenyl is selected from the group consisting of dimethylaminophenyl, diethylaminophenyl, dipropylaminophenyl, dibutylaminophenyl, and dibenzylaminophenyl.

5. An electrophotographic photosensitive member of claim 4, wherein said dialkylamino is diethylamino.

6. An electrophotographic photosensitive member of claim 1, wherein said  $R_1$  is a heterocyclic residue selected from the group consisting of pyridyl, quinolyl, carbazolyl, and imidazolyl.

7. An electrophotographic photosensitive member of claim 6, wherein said  $R_1$  is carbazolyl.

8. An electrophotographic photosensitive member of claim 1, wherein said  $X_1$  is a heterocyclic residue selected from the group consisting of 2-pyridyl, 3-pyridyl, 4-pyridyl, 6-methoxy-2-pyridyl, 2-quinolyl, 4-quinolyl, 2-lepidyl, 3-carbazolyl, and 9-ethyl-3-carbazolyl.

9. An electrophotographic photosensitive member comprising a layer which includes a charge generating material, a binder and at least one pyrazoline compound of the formula:



5

R<sub>1</sub> is a substituted or unsubstituted aryl or heterocyclic residue;  
 R<sub>4</sub> is hydrogen, a halogen, or a substituted or unsubstituted alkyl or aryl;  
 R<sub>11</sub> is a substituted or unsubstituted alkyl;  
 R<sub>12</sub> is hydrogen, a halogen or an organic monovalent residue;  
 Z is



or —CH=CH—, wherein R<sub>13</sub> and R<sub>14</sub> are each substituted or unsubstituted alkyl;  
 n is 0 or 1; and  
 l is an integer of 1 to 4.

\* \* \* \* \*

15  
 wherein X<sub>1</sub> is a substituted or unsubstituted heterocyclic residue selected from the group consisting of substituted or unsubstituted pyridyl, quinolyl, carbazolyl, furyl, imidazolyl, oxazolyl and isoxazolyl;

20

25

30

35

40

45

50

55

60

65